



US006423481B1

(12) **United States Patent**  
Simpson et al.

(10) **Patent No.:** US 6,423,481 B1  
(45) **Date of Patent:** Jul. 23, 2002

(54) **HIGH SPEED PHOTOTHERMOGRAPHIC MATERIALS WITH COMBINED CHEMICAL SENSITIZERS AND METHODS OF USING SAME**

(75) Inventors: **Sharon M. Simpson**, Lake Elmo; **David R. Whitcomb**; **Steven M. Shor**, both of Woodbury, all of MN (US)

(73) Assignee: **Eastman Kodak Company**, Rochester, NY (US)

(\*) Notice: Subject to any disclaimer, the term of this patent is extended or adjusted under 35 U.S.C. 154(b) by 0 days.

(21) Appl. No.: **09/768,094**

(22) Filed: **Jan. 23, 2001**

(51) **Int. Cl.<sup>7</sup>** ..... G03C 1/498; G03C 1/09

(52) **U.S. Cl.** ..... 430/350; 430/510; 430/517; 430/600; 430/603; 430/604; 430/605; 430/619

(58) **Field of Search** ..... 430/350, 510, 430/600, 517, 603, 523, 604, 605, 619

(56) **References Cited**

U.S. PATENT DOCUMENTS

|               |         |                    |
|---------------|---------|--------------------|
| 2,597,856 A   | 5/1952  | Damschroder        |
| 2,597,915 A   | 5/1952  | Yutzy et al.       |
| 2,642,361 A   | 6/1953  | Damschroder et al. |
| 3,503,749 A   | 3/1970  | Tavernier et al.   |
| 4,030,930 A   | 6/1977  | Sashihara et al.   |
| 4,036,650 A   | 7/1977  | Hasegawa et al.    |
| 4,621,041 A   | 11/1986 | Saikawa et al.     |
| 5,001,042 A   | 3/1991  | Hasebe             |
| 5,049,485 A   | 9/1991  | Deaton             |
| 5,220,030 A   | 6/1993  | Deaton             |
| 5,252,455 A   | 10/1993 | Deaton             |
| 5,362,470 A   | 11/1994 | Masutomi et al.    |
| 5,391,727 A   | 2/1995  | Deaton             |
| 5,756,728 A * | 5/1998  | Lok ..... 430/600  |
| 5,759,761 A   | 6/1998  | Lughington et al.  |
| 5,858,637 A   | 1/1999  | Eshelman et al.    |
| 5,891,615 A   | 4/1999  | Winslow et al.     |
| 6,100,022 A   | 8/2000  | Inoue et al.       |

FOREIGN PATENT DOCUMENTS

|    |              |         |
|----|--------------|---------|
| EP | 0 911 692 A2 | 4/1999  |
| JP | 4-257853     | 9/1992  |
| JP | 4-308843     | 10/1992 |
| JP | 11-194447    | 11/1999 |

SU 1153694 A1 4/1983

OTHER PUBLICATIONS

JP 11-65,020—Aug. 14, 1997—Summary.

JP 11194447—Abstract.

JP 4308843—Abstract.

SU 1153694—Abstract.

Gajendragad et al, "Complexing Behaviour of 5-Amino-1,3,4-Thiazole-2-thiol. II. Complexes of Ni(II), Rh(II), Pt(II), Au(III) and Cu(II)", Bull. Chem. Soc. Jap., 48, pp. 1024-1029 (1975).

Fabretti et al., "Silver (I) and Gold (I) Complexes of Rhodanine" Transition Met. Chem., 2, pp 224-227 (1977). Siew et al, "The Structure of Aold (4—2-Thione-5,5 Dimethylthiazolidine)" J. Inorg. Nucl. Chem., 38, pp 7-11 (1976).

Fabretti et al, "Reaction Products between Gold (III) Bro-mide and Tetramethylthiourea: Dibromobis(tetramethylthiourea)gold (III) . . . "J. Chem. Soc., Dalton Trans., pp 3091-3093 (1990).

Deaton et al., "Gold (I)combination compounds with mesionic thio ligands and the crystal and molecular structure of bis(1,4,5-trimethyl-1,2,4-triazolium-3-thiolate) gold(I) tetrafluoroborate", J. Chem. Soc., Dalton Trans., pp 3163-6167 (1999).

\* cited by examiner

Primary Examiner—Thorl Chea

(74) Attorney, Agent, or Firm—J. Lanny Tucker; Louis M. Leichter

(57) **ABSTRACT**

Photothermographic materials have increased photospeed provided by gold(III)-containing chemical sensitizers that are used combination with sulfur- and/or tellurium-containing chemical sensitizers. Increased photographic speed is achieved with minimal increase in  $D_{min}$ . The gold(III)-containing chemical sensitizers are represented by the following Structure GOLD:



GOLD

wherein L' represents the same or different ligands, each ligand comprising at least one heteroatom that is capable of forming a bond with gold, Y is an anion, r is an integer of from 1 to 8, and q is an integer of from 0 to 3.

**46 Claims, No Drawings**

**HIGH SPEED PHOTOTHERMOGRAPHIC  
MATERIALS WITH COMBINED CHEMICAL  
SENSITIZERS AND METHODS OF USING  
SAME**

**FIELD OF THE INVENTION**

This invention relates to thermally developable imaging materials such as photothermographic materials that exhibit high speed imaging characteristics. In particular, this invention relates to the use of certain gold(III) compounds as chemical sensitizers in combination with sulfur or tellurium chemical sensitizers in photothermographic materials to provide increased photothermographic speed. This invention also relates to methods of imaging using these photothermographic materials and methods for their preparation.

**BACKGROUND OF THE INVENTION**

Photothermographic imaging materials that are developed with heat and without liquid development have been known in the art for many years. Such materials are used in a recording process wherein an image is formed by imagewise exposure of the photothermographic material to specific electromagnetic radiation (for example, visible, ultraviolet, or infrared radiation) and developed by the use of thermal energy. These materials, also known as "dry silver" materials, generally comprise a support having coated thereon: (a) photosensitive catalyst (such as silver halide) that upon such exposure provides a latent image in exposed grains that are capable of acting as a catalyst for the subsequent formation of a silver image in a development step, (b) a relatively or completely non-photosensitive source of reducible silver ions, (c) a reducing composition (usually including a developer) for the reducible silver ions, and (d) a hydrophilic or hydrophobic binder. The latent image is then developed by application of thermal energy.

In such materials, the photosensitive catalyst is generally a photographic type photosensitive silver halide that is considered to be in catalytic proximity to the non-photosensitive source of reducible silver ions. Catalytic proximity requires intimate physical association of these two components either prior to or during the thermal image development process so that when silver atoms ( $\text{Ag}^0$ )<sub>n</sub>, also known as silver specks, clusters, nuclei or latent image, are generated by irradiation or light exposure of the photosensitive silver halide, those silver atoms are able to catalyze the reduction of the reducible silver ions within a catalytic sphere of influence around the silver atoms [D. H. Klosterboer, *Imaging Processes and Materials*, (Neblette's Eighth Edition), Sturge, Walworth & Shepp (Eds.), Van Nostrand-Reinhold, New York, Chapter 9, pages 279-291, 1989]. It has long been understood that silver atoms act as a catalyst for the reduction of silver ions, and that the photosensitive silver halide can be placed in catalytic proximity with the non-photosensitive source of reducible silver ions in a number of different ways (see, for example, *Research Disclosure*, June 1978, item 17029). Other photosensitive materials, such as titanium dioxide, cadmium sulfide, and zinc oxide have also been reported to be useful in place of silver halide as the photocatalyst in photothermographic materials [see for example, Shepard, *J. Appl. Photog. Eng.* 1982, 8(5), 210-212, Shigeo et al., *Nippon Kagaku Kaishi*, 1994, 11, 992-997, and FR 2,254,047 (Robillard)].

The photosensitive silver halide may be made "in situ," for example by mixing an organic or inorganic halide-containing source with a source of reducible silver ions to

achieve partial metathesis and thus causing the in-situ formation of silver halide (AgX) grains throughout the silver source [see, for example, U.S. Pat. No. 3,457,075 (Morgan et al.)].

5 The silver halide may also be "preformed" and prepared by an "ex situ" process whereby the silver halide (AgX) grains are prepared and grown separately. With this technique, one has the possibility of controlling the grain size, grain size distribution, dopant levels, and composition much more precisely, so that one can impart more specific properties to both the silver halide grains and the photothermographic material. The preformed silver halide grains may be introduced prior to and be present during the formation of the source of reducible silver ions. Co-precipitation of the silver halide and the source of reducible silver ions provides a more intimate mixture of the two materials [see for example U.S. Pat. No. 3,839,049 (Simons)]. Alternatively, the preformed silver halide grains may be added to and physically mixed with the source of reducible silver ions.

10 The non-photosensitive source of reducible silver ions is a material that contains reducible silver ions. Typically, the preferred non-photosensitive source of reducible silver ions is a silver salt of a long chain aliphatic carboxylic acid having from 10 to 30 carbon atoms, or mixtures of such salts. Such acids are also known as "fatty acids". Silver salts 15 of other organic acids or other organic compounds, such as silver imidazoles, silver tetrazoles, silver benzotriazoles, silver benzotetrazoles, silver benzothiazoles and silver acetylides have also been proposed. U.S. Pat. No. 4,260,677 (Winslow et al.) discloses the use of complexes of various 20 inorganic or organic silver salts.

25 In photothermographic materials, exposure of the photographic silver halide to light produces small clusters containing silver atoms ( $\text{Ag}^0$ )<sub>n</sub>. The imagewise distribution of these clusters, known in the art as a latent image, is generally 30 not visible by ordinary means. Thus, the photosensitive material must be further developed to produce a visible image. This is accomplished by the reduction of silver ions that are in catalytic proximity to silver halide grains bearing the silver-containing clusters of latent image. This produces 35 a black-and-white image. The non-photosensitive silver source is catalytically reduced to form the visible black-and-white negative image while much of the silver halide, generally, remains as silver halide and is not reduced.

40 In photothermographic materials, the reducing agent for the reducible silver ions, often referred to as a "developer," 45 may be any compound that, in the presence of the latent image, can reduce silver ion to metallic silver and is preferably of relatively low activity until it is heated to a temperature sufficient to cause the reaction. A wide variety 50 of classes of compounds have been disclosed in the literature that function as developers for photothermographic materials. At elevated temperatures, the reducible silver ions are reduced by the reducing agent. In photothermographic materials, upon heating, this reaction occurs preferentially in 55 the regions surrounding the latent image. This reaction produces a negative image of metallic silver having a color that ranges from yellow to deep black depending upon the presence of toning agents and other components in the imaging layer(s).

60 **Differences Between Photothermography and Photography**  
The imaging arts have long recognized that the field of photothermography is clearly distinct from that of photography. Photothermographic materials differ significantly from conventional silver halide photographic materials that require processing with aqueous processing solutions.

65 As noted above, in photothermographic imaging materials, a visible image is created by heat as a result of the

reaction of a developer incorporated within the material. Heating at 50° C. or more is essential for this dry development. In contrast, conventional photographic imaging materials require processing in aqueous processing baths at more moderate temperatures (from 30° C. to 50° C.) to provide a visible image.

In photothermographic materials, only a small amount of silver halide is used to capture light and a non-photosensitive source of reducible silver ions (for example a silver carboxylate) is used to generate the visible image using thermal development. Thus, the imaged photosensitive silver halide serves as a catalyst for the physical development process involving the non-photosensitive source of reducible silver ions and the incorporated reducing agent. In contrast, conventional wet-processed, black-and-white photographic materials use only one form of silver (that is, silver halide) that, upon chemical development, is itself converted into the silver image, or that upon physical development requires addition of an external silver source (or other reducible metal ions that form black images upon reduction to the corresponding metal). Thus, photothermographic materials require an amount of silver halide per unit area that is only a fraction of that used in conventional wet-processed photographic materials.

In photothermographic materials, all of the "chemistry" for imaging is incorporated within the material itself. For example, such materials include a developer (that is, a reducing agent for the reducible silver ions) while conventional photographic materials usually do not. Even in so-called "instant photography," the developer chemistry is physically separated from the photosensitive silver halide until development is desired. The incorporation of the developer into photothermographic materials can lead to increased formation of various types of "fog" or other undesirable sensitometric side effects. Therefore, much effort has gone into the preparation and manufacture of photothermographic materials to minimize these problems during the preparation of the photothermographic emulsion as well as during coating, use, storage, and post-processing handling.

Moreover, in photothermographic materials, the unexposed silver halide generally remains intact after development and the material must be stabilized against further imaging and development. In contrast, silver halide is removed from conventional photographic materials after solution development to prevent further imaging (that is in the aqueous fixing step).

In photothermographic materials, the binder is capable of wide variation and a number of binders (both hydrophilic and hydrophobic) are useful. In contrast, conventional photographic materials are limited almost exclusively to hydrophilic colloidal binders such as gelatin.

Because photothermographic materials require dry thermal processing, they present distinctly different problems and require different materials in manufacture and use, compared to conventional, wet-processed silver halide photographic materials. Additives that have one effect in conventional silver halide photographic materials may behave quite differently when incorporated in photothermographic materials where the underlying chemistry is significantly more complex. The incorporation of such additives as, for example, stabilizers, antifoggants, speed enhancers, supersensitizers, and spectral and chemical sensitizers in conventional photographic materials is not predictive of whether such additives will prove beneficial or detrimental in photothermographic materials. For example, it is not uncommon for a photographic antifog useful in conven-

tional photographic materials to cause various types of fog when incorporated into photothermographic materials, or for supersensitizers that are effective in photographic materials to be inactive in photothermographic materials.

These and other distinctions between photothermographic and photographic materials are described in *Imaging Processes and Materials* (Nebblette's Eighth Edition), noted above, *Unconventional Imaging Processes*, E. Brinckman et al. (Eds.), The Focal Press, London and New York, 1978, pp. 74-75, C-f. Zou et al., *J. Imaging Sci. Technol.* 1996, 40, pp. 94-103, and in M. R. V. Sahyun, *J. Imaging Sci. Technol.* 1998, 42, 23.

#### Problem to be Solved

One of the challenges in the use of photothermographic materials is attaining sufficient photothermographic speed in such materials that are also compatible with conventional imaging sources.

Each of the pure photographic silver halides (silver chloride, silver bromide and silver iodide) has its own natural response to radiation, in both wavelength and speed, within the UV, near UV and blue regions of the electromagnetic spectrum. Mixtures of silver halides (for example, silver bromochloroiodide, silver chloroiodide, silver chlorobromide, and silver iodobromide) also have their own natural sensitivities within the UV and blue regions of the electromagnetic spectrum. Thus, silver halide grains, when composed of only silver and halogen atoms have defined levels of sensitivity depending upon the levels of specific halogens, crystal morphology (shape and structure of the crystals or grains) and other characteristics, such as, for example, crystal defects, stresses, and dislocations, and dopants, incorporated within or on the crystal lattice of the silver halide. These features may or may not have been readily controlled or purposely introduced to affect emulsion sensitometry.

The efforts to influence silver halide grain speed in conventional wet-processed silver halide emulsions generally fall within the investigation of crystal composition, morphology or structure (all briefly described above), or the use of dopants, spectral sensitizers, supersensitizers, reduction sensitizers, and chemical sensitizers (particularly sulfur sensitizers).

Spectral sensitization is the addition of a compound (usually a dye) to silver halide grains that absorbs radiation at wavelengths (UV, visible or IR) other than those to which the silver halide is naturally sensitive, or that absorbs radiation more efficiently than silver halide (even within the regions of silver halide's natural sensitivity). It is generally recognized that spectral sensitizers extend the responses of photosensitive silver halide to longer wavelengths. After absorption of the radiation, these compounds transfer energy or electrons to the silver halide grains to cause the necessary local photoinduced reduction of silver (I) to silver (0).

Supersensitization is a process whereby the speed of spectrally sensitized silver halide is increased by the addition of still another compound that may or may not be a dye. This is not merely an additive effect of the two compounds (spectral sensitizer and supersensitizer).

Reduction sensitization is a type of chemical sensitization (described in more detail in the following paragraphs) in which other chemical species (not sulfur-containing) are deposited onto, or reacted with, the silver halide grains during grain growth and finishing. Compounds used for this purpose act as reducing agents on the silver halide grains and include, but are not limited to, stannous chloride, hydrazine, ethanolamine, and thioureaoxide.

Chemical sensitization (generally sulfur-sensitization) is a process, during or after silver halide crystal formation, in

which sensitization centers [for example, silver sulfide clusters such as  $(Ag_2S)_n$ ] are introduced onto the individual silver halide grains. For example, silver sulfide specks can be introduced by direct reaction of sulfur-contributing compounds with the silver halide during various stages or after completion of silver halide grain growth. These specks usually function as shallow electron traps for the preferential formation of a latent image center. Other chalcogens (Se and Te) can function similarly. The presence of these specks increases the speed or sensitivity of the resulting silver halide grains to radiation. Sulfur-contributing compounds useful for this purpose include thiosulfates (such as sodium thiosulfate) and various thioureas (such as allyl thiourea, thiourea, triethyl thiourea and 1,1'-diphenyl-2-thiourea) as described for example, by Sheppard et al., *J. Franklin Inst.*, 1923, pp. 196, 653 and 673, C. E. K. Mees and T. H. James, *The Theory of the Photographic Process*, 4<sup>th</sup> Edition, 1977, pp. 152-3, and Tani, T., *Photographic Sensitivity: Theory and Mechanisms*, Oxford University Press, N.Y., 1995, pp. 167-176.

Another method of chemical sensitization is achieved by oxidative decomposition of a sulfur-containing spectral sensitizing dye in a photothermographic emulsion as described in U.S. Pat. No. 5,891,615 (Winslow et al.).

Chemical sensitization to increase photospeed has also been achieved by treating the silver halide grains with gold-containing ions such as tetrachloroaurate (III) or dithiocyanatoaurate (I). Preferably, the gold compounds are added in the later stages of silver halide grain formation such as during ripening. Platinum and palladium compounds are also known to have similar effects. In comparison, iridium, rhodium, and ruthenium compounds are generally used to control contrast and/or high intensity reciprocity effects rather than to increase speed.

It is well known that the various speed enhancing means just described can be used in combination as the situation requires.

As noted above, in photothermographic emulsions, the photosensitive silver halide must be in catalytic proximity to (or in reactive association with) the non-photosensitive source of reducible silver ions. Because of the different emulsion making procedures and chemical environments of photothermographic emulsions, the effects achieved by compounds (such as chemical sensitizers) in conventional photographic emulsions are not necessarily possible in photothermographic emulsions.

For example, in photothermographic emulsions, two types of chemical sensitization have been used to increase speed: (a) chemical sensitization of preformed silver halide grains that are then mixed into the solution containing reducible silver ions in some manner, and (b) chemical sensitization of preformed silver halide grains that are already in intimate contact with the reducible silver ions.

In the first approach (a), many of the traditional methods (used for photographic emulsions) can be used, but for the second approach (b), quite specific methods and unique compounds are often needed. Regardless of which approach is used, there is considerable difficulty in attaining additional speed while maintaining low fog ( $D_{min}$ ).

The use of sodium thiosulfate, triarylpophosphine selenide and dibenzoyl ditelluride, or mixtures thereof, as chemical sensitizers for photothermographic materials is also known. For example, U.S. Pat. No. 4,639,414 (Sakaguchi) describes the use of sodium thiosulfate to decrease fog and loss of sensitivity upon storage in a silver benzotriazole, gelatin-based photothermographic emulsion. The light-sensitive silver halide is said to be chemically sensitized in the presence

of a sensitizing dye that is added after the formation of silver halide but before the completion of chemical sensitization.

Various sulfur-containing chemical sensitizers are also known in the art and described in numerous references. For example, U.S. Pat. No. 4,810,626 (Burgmaier et al.), U.S. Pat. No. 4,213,784 (Ikenoue et al.), and U.S. Pat. No. 5,843,632 (Eshelman et al.) describe various thioureas that may be used in this manner in certain emulsion conditions.

Another useful class of chemical sensitizers is the tetra-substituted thiourea compounds described in copending and commonly assigned U.S. Ser. No. 09/667,748 (filed Sep. 21, 2000 by Lynch, Simpson, Shor, Willett, and Zou). These compounds are shown to provide increased photospeed with minimal loss in  $D_{min}$ .

Tellurium chemical sensitization of photothermographic materials has also been reported. For example, U.S. Pat. No. 6,025,122 (Sakai et al.) and U.S. Pat. No. 5,968,725 (Katoh et al.) describe the use of conventional tellurides such as dibenzoyl ditelluride, and other tellurium compounds as chemical sensitizers. It is also known to use dibenzoyl ditelluride in combination with other chemical sensitizers such as sodium thiosulfate, pentafluorophenyl diphenyl phosphine selenide and chloroauric acid [that is a Au(I) compound] in thermally developable materials.

Particularly useful tellurium chemical sensitizers are described and claimed in copending and commonly assigned U.S. Ser. No. 09/746,400 (filed Dec. 21, 2000 by Lynch, Opatz, Shor, Simpson, Willett, and Gysling,) and entitled "High Speed Photothermographic Materials Containing Tellurium Compounds and Methods of Using Same" (Attorney Docket 80836/JLT), incorporated herein by reference.

Gold has also been used in conventional photographic materials as a chemical sensitizer [for example, as described in U.S. Pat. No. 5,220,030 (Deaton)]. While gold may be generally added to formulations as Au(III), for example as a  $KAuX_4$  compound, it is believed that Au(I) is the active species in such uses (see for example, Tani, *Photographic Sensitivity*, Oxford University Press, 1995). U.S. Pat. No. 5,858,637 (Eshelman et al.) also describes various Au(I) compounds that can be used as chemical sensitizers in photothermographic compositions and materials. Particularly useful are sulfur-containing 1,1,3,3-tetrasubstituted thiourea compounds having an acid group with an acid dissociation constant ( $pK_a$ ) of less than 7.

Photothermographic materials are constantly being redesigned to meet ever-increasing performance, storage, and manufacturing demands raised by customers, regulators, and manufacturers. One of these demands is increased photospeed without a significant increase in fog ( $D_{min}$ ) or a loss in  $D_{max}$ .

## SUMMARY OF THE INVENTION

The present invention relates to our discovery that the combination of certain gold(III)-containing compounds with either sulfur- or tellurium-containing compounds or with a combination of one or more of sulfur- and one or more tellurium-containing compounds provides chemical sensitization of photothermographic materials. The photothermographic materials thus prepared have increased photospeed without significant increase in  $D_{min}$ .

The present invention provides the desired benefits with a photothermographic material comprising a support having thereon one or more layers comprising a binder and in reactive association:

- 65 a. photosensitive silver halide grains,
- b. a non-photosensitive source of reducible silver ions, and

- c. a reducing composition for the reducible silver ions, wherein the photosensitive silver halide grains have been chemically sensitized with a combination of chemical sensitizers that consists essentially of a sulfur- or tellurium-containing compound, and a gold(III)-containing compound that is represented by the following Structure GOLD:



GOLD

wherein L' represents the same or different ligands, each ligand comprising a heteroatom that is capable of forming a bond with gold, Y is an anion, r is an integer of from 1 to 8, and q is an integer of from 0 to 3.

Further, a method of this invention for forming a visible image comprises:

- A) imagewise exposing the photothermographic material described above to electromagnetic radiation to form a latent image, and
  - B) simultaneously or sequentially, heating the exposed photothermographic material to develop the latent image into a visible image.
- In some embodiments of this invention to provide an image, the photothermographic material has a transparent support and the method of this invention further includes:
- C) positioning the exposed and heat-developed photothermographic material with a visible image therein between a source of imaging radiation and an imageable material that is sensitive to the imaging radiation, and
  - D) thereafter exposing the imageable material to the imaging radiation through the visible image in the exposed and heat-developed photothermographic material to provide a visible image in the imageable material.

In still another embodiment of this invention, a method for preparing a photothermographic emulsion comprises:

- A) providing a photothermographic emulsion comprising photosensitive silver halide grains and a non-photosensitive source of reducible silver ions, and
- B) positioning one or more gold(III)-containing chemical sensitizers and one or more sulfur- or tellurium-containing chemical sensitizers on or around the photosensitive silver halide grains, the one or more gold (III)-containing chemical sensitizers being represented by the Structure GOLD noted above.

Moreover, another method of preparing a photothermographic emulsion comprises:

- A) providing photosensitive silver halide grains,
- B) providing a photothermographic emulsion of the photosensitive silver halide grains and a non-photosensitive source of reducible silver ions, and
- C) prior to, during, or immediately following either or both of steps A and B, chemically sensitizing the photosensitive silver halide grains with a combination of chemical sensitizers that consists essentially of a gold(III)-containing compound and a sulfur- or tellurium-containing compound, the gold(III)-containing compound being represented by the Structure GOLD noted above.

The combination of chemical sensitizing compounds described for use in the photothermographic materials of this invention has a number of useful properties. For example, the chemical sensitizing compounds can easily be prepared

in good yield, are stable in air, and are resistant to hydrolysis. Moreover, they are soluble in a range of useful coating solvents. This allows them to be included easily in the imaging element formulations.

- 5 The speed increasing ability of the combination of chemical sensitizers described herein was not anticipated from the teaching in the prior art. Moreover, prior art chemical sensitizers have generally not produced speed enhancement while maintaining high  $D_{max}$  and low  $D_{min}$ . It was also apparent to us that using gold(III)-, sulfur- or tellurium-containing compounds alone did not provide the best results. Quite unexpectedly, we discovered that certain gold(III)-containing compounds provide the noted advantages only in combination with a sulfur- or tellurium-containing chemical 10 sensitizing compound. This combination of compounds was also unexpectedly better than a combination of gold(I)-containing compound and a sulfur- or tellurium-containing compound, or similar combinations of gold(III) compounds outside of the scope of the Structure GOLD.

#### DETAILED DESCRIPTION OF THE INVENTION

The photothermographic materials of this invention can be used, for example, in conventional black-and-white photothermography, in electronically generated black-and-white hardcopy recording, in the graphic arts area (for example imagesetting and phototypesetting), in the manufacture of printing plates, in proofing, in microfilm applications, and in radiographic imaging. Furthermore, the absorbance of these photothermographic materials between 350 and 450 nm is desirably low (less than 0.5) to permit their use in graphic arts applications such as contact printing, proofing, and duplicating ("duping").

In the photothermographic materials of this invention, the 35 components needed for imaging can be in one or more layers. The layer(s) that contain the photosensitive photocatalyst (such as a photosensitive silver halide) or non-photosensitive source of reducible silver ions, or both, are referred to herein as photothermographic emulsion layer(s). 40 The photocatalyst and the non-photosensitive source of reducible silver ions are in catalytic proximity (or in reactive association with each other) and preferably are in the same layer.

Various layers are usually disposed on the "backside" 45 (non-emulsion side) of the materials, including antihalation layer(s), protective layers, antistatic layers, conducting layers, and transport enabling layers.

Various layers are also usually disposed on the "frontside" 50 or emulsion side of the support, including protective topcoat layers, primer layers, interlayers, opacifying layers, anti-static layers, antihalation layers, acutance layers, auxiliary layers, and others readily apparent to one skilled in the art.

The present invention also provides a process for the formation of a visible image (usually a black-and-white image) by first exposing to electromagnetic radiation and thereafter heating the inventive photothermographic material. In one embodiment, the present invention provides a process comprising:

- A) imagewise exposing the photothermographic material of this invention to electromagnetic radiation to which the photocatalyst (for example, a photosensitive silver halide) of the material is sensitive, to generate a latent image, and
- B) simultaneously or sequentially, heating the exposed material to develop the latent image into a visible image.

This visible image can also be used as a mask for exposure of other photosensitive imageable materials, such as graphic arts films, proofing films, printing plates and circuit board films, that are sensitive to suitable imaging radiation (for example UV radiation). This can be done by imaging an imageable material (such as a photopolymer, a diazo material, a photoresist, or a photosensitive printing plate) through the exposed and heat-developed photothermographic material of this invention using steps C) and D) noted above.

When the photothermographic materials of this invention are heat-developed as described below in a substantially water-free condition after, or simultaneously with, image-wise exposure, a silver image (preferably a black-and-white silver image) is obtained. The photothermographic material may be exposed in step A using ultraviolet, visible, infrared or laser radiation using an infrared laser, a laser diode, an infrared laser diode, a light-emitting screen, CRT tube, a light-emitting diode, or other light or radiation source readily apparent to one skilled in the art.

#### Definitions

As used herein:

In the descriptions of the photothermographic materials of the present invention, "a" or "an" component refers to "at least one" of that component. For example, the gold compounds described herein for chemical sensitization can be used individually or in combination.

Heating in a substantially water-free condition as used herein, means heating at a temperature of from about 50° to about 250° C. with little more than ambient water vapor present. The term "substantially water-free condition" means that the reaction system is approximately in equilibrium with water in the air and water for inducing or promoting the reaction is not particularly or positively supplied from the exterior to the material. Such a condition is described in T. H. James, *The Theory of the Photographic Process*, Fourth Edition, Macmillan 1977, p. 374.

"Photothermographic material(s)" means a construction comprising at least one photothermographic emulsion layer or a photothermographic set of layers (wherein the silver halide and the source of reducible silver ions are in one layer and the other essential components or desirable additives are distributed, as desired, in an adjacent coating layer) and any supports, topcoat layers, image-receiving layers, blocking layers, antihalation layers, subbing or priming layers. These materials also include multilayer constructions in which one or more imaging components are in different layers, but are in "reactive association" so that they readily come into contact with each other during imaging and/or development. For example, one layer can include the non-photosensitive source of reducible silver ions and another layer can include the reducing composition, but the two reactive components are in reactive association with each other.

"Emulsion layer", "imaging layer", or "photothermographic emulsion layer" means a layer of a photothermographic material that contains the photosensitive silver halide and/or non-photosensitive source of reducible silver ions. It can also mean a layer of the photothermographic material that contains, in addition to the photosensitive silver halide and/or non-photosensitive source of reducible ions, additional essential components and/or desirable additives. These layers are usually on what is known as the "frontside" of the support.

"Ultraviolet region of the spectrum" refers to that region of the spectrum less than or equal to 410 nm, and preferably from about 100 nm to about 410 nm, although parts of these ranges may be visible to the naked human eye. More

preferably, the ultraviolet region of the spectrum is the region of from about 190 to about 405 nm.

"Visible region of the spectrum" refers to that region of the spectrum of from about 400 nm to about 750 nm.

"Short wavelength visible region of the spectrum" refers to that region of the spectrum of from about 400 nm to about 450 nm.

"Red region of the spectrum" refers to that region of the spectrum of from about 600 nm to about 750 nm.

"Infrared region of the spectrum" refers to that region of the spectrum of from about 750 nm to about 1400 nm.

"Non-photosensitive" means not intentionally light sensitive.

The sensitometric terms "photospeed" or "photographic speed",  $D_{min}$ , and  $D_{max}$  have conventional definitions known in the imaging arts.

"Transparent" means capable of transmitting visible light or imaging radiation without appreciable scattering or absorption.

As is well understood in this art, for the gold-containing compounds herein, substitution is not only tolerated, but is often advisable and various substituents are anticipated on the compounds used in the present invention. Thus, when a compound is referred to as "having the structure" of a given

formula, any substitution that does not alter the bond structure of the formula or the shown atoms within that structure is included within the formula, unless such substitution is specifically excluded by language (such as "free of carboxy-substituted alkyl"). For example, where a benzene ring structure is shown (including fused ring structures), substituent groups may be placed on the benzene ring structure, but the atoms making up the benzene ring structure may not be replaced.

As a means of simplifying the discussion and recitation of

certain substituent groups, the term "group" refers to chemical species that may be substituted as well as those that are not so substituted. Thus, the term "group," such as "alkyl group" is intended to include not only pure hydrocarbon alkyl chains, such as methyl, ethyl, propyl, t-butyl, cyclohexyl, iso-octyl, octadecyl and the like, but also alkyl chains bearing substituents known in the art, such as hydroxyl, alkoxy, phenyl, halogen atoms (F, Cl, Br, and I), cyano, nitro, amino, carboxy and the like. For example, alkyl group includes ether and thioether groups (for example  $CH_3—CH_2—CH_2—O—CH_2—$ ), haloalkyl, nitroalkyl, carboxyalkyl, hydroxyalkyl, sulfoalkyl, and other groups readily apparent to one skilled in the art. Substituents that adversely react with other active ingredients, such as very strongly electrophilic or oxidizing substituents, would, of course, be excluded by the ordinarily skilled artisan as not being inert or harmless.

*Research Disclosure* is a publication of Kenneth Mason Publications Ltd., Dudley House, 12 North Street, Emsworth, Hampshire PO10 7DQ England (also available from Emsworth Design Inc., 147 West 24th Street, New York, N.Y. 10011).

Other aspects, advantages, and benefits of the present invention are apparent from the detailed description, examples, and claims provided in this application.

#### The Photocatalyst

As noted above, the photothermographic materials of the present invention include one or more photocatalysts in the photothermographic emulsion layer(s). Useful photocatalysts are typically silver halides such as silver bromide, silver iodide, silver chloride, silver bromoiodide, silver chlorobromoiodide, silver chlorobromide, and others readily apparent to one skilled in the art. Mixtures of silver halides

can also be used in any suitable proportion. Silver bromide and silver bromoiodide are more preferred, with the latter silver halide having up to 10 mol % silver iodide.

The shape of the photosensitive silver halide grains used in the present invention is in no way limited. The silver halide grains may have any crystalline habit including, but not limited to, cubic, octahedral, rhombic dodecahedral, orthorhombic, tetrahedral, other polyhedral, laminar, twinned, platelet, or tabular morphologies and may have epitaxial growth of crystals thereon. If desired, a mixture of these crystals can be employed. Silver halide grains having cubic and tabular morphology are preferred.

The silver halide grains may have a uniform ratio of halide throughout. They may have a graded halide content, with a continuously varying ratio of, for example, silver bromide and silver iodide or they may be of the core-shell type, having a discrete core of one halide ratio, and a discrete shell of another halide ratio. Core-shell silver halide grains useful in photothermographic materials and methods of preparing these materials are described for example in U.S. Pat. No. 5,382,504 (Shor et al.) incorporated herein by reference. Iridium and/or copper doped core-shell and non-core-shell grains are described in U.S. Pat. No. 5,434,043 (Zou et al.) and U.S. Pat. No. 5,939,249 (Zou), incorporated herein by reference.

The photosensitive silver halide can be added to (or formed within) the emulsion layer(s) in any fashion as long as it is placed in catalytic proximity to the non-photosensitive source of reducible silver ions.

It is preferred that the silver halides be preformed and prepared by an ex-situ process. The silver halide grains prepared ex-situ may then be added to and physically mixed with the non-photosensitive source of reducible silver ions. It is more preferable to form the source of reducible silver ions in the presence of ex-situ-prepared silver halide. In this process, the source of reducible silver ions, such as a long chain fatty acid silver carboxylate (commonly referred to as a silver "soap"), is formed in the presence of the preformed silver halide grains. Co-precipitation of the reducible source of silver ions in the presence of silver halide provides a more intimate mixture of the two materials [see, for example U.S. Pat. No. 3,839,049 (Simons)]. Materials of this type are often referred to as "preformed soaps."

The silver halide grains used in the imaging formulations can vary in average diameter of up to several micrometers ( $\mu\text{m}$ ) depending on their desired use. Preferred silver halide grains are those having an average particle size of from about 0.01 to about 1.5  $\mu\text{m}$ , more preferred are those having an average particle size of from about 0.03 to about 1.0  $\mu\text{m}$ , and most preferred are those having an average particle size of from about 0.05 to about 0.8  $\mu\text{m}$ . Those of ordinary skill in the art understand that there is a finite lower practical limit for silver halide grains that is partially dependent upon the wavelengths to which the grains are spectrally sensitized. Such a lower limit, for example, is typically from about 0.01 to about 0.005  $\mu\text{m}$ .

The average size of the photosensitive doped silver halide grains is expressed by the average diameter if the grains are spherical, and by the average of the diameters of equivalent circles for the projected images if the grains are cubic or in other non-spherical shapes.

Grain size may be determined by any of the methods commonly employed in the art for particle size measurement. Representative methods are described by in "Particle Size Analysis," ASTM Symposium on Light Microscopy, R. P. Loveland, 1955, pp. 94-122, and in C. E. K. Mees and T. H. James, *The Theory of the Photographic Process*, Third

Edition, Chapter 2, Macmillan Company, 1966. Particle size measurements may be expressed in terms of the projected areas of grains or approximations of their diameters. These will provide reasonably accurate results if the grains of interest are substantially uniform in shape.

Preformed silver halide emulsions used in the material of this invention can be prepared by aqueous or organic processes and can be unwashed or washed to remove soluble salts. In the latter case, the soluble salts can be removed by ultrafiltration, by chill setting and leaching, or by washing the coagulum [for example, by the procedures described in U.S. Pat. No. 2,618,556 (Hewitson et al.), U.S. Pat. No. 2,614,928 (Yutzy et al.), U.S. Pat. No. 2,565,418 (Yackel), U.S. Pat. No. 3,241,969 (Hart et al.) and U.S. Pat. No. 2,489,341 (Waller et al.)].

It is also effective to use an in situ process in which a halide-containing compound is added to an organic silver salt to partially convert the silver of the organic silver salt to silver halide. The halogen-containing compound can be inorganic (such as zinc bromide or lithium bromide) or organic (such as N-bromosuccinimide).

Additional methods of preparing these silver halide and organic silver salts and manners of blending them are described in *Research Disclosure*, June 1978, item 17029, 25 U.S. Pat. No. 3,700,458 (Lindholm) and U.S. Pat. No. 4,076,539 (Ikenoue et al.), and JP Applications 13224/74, 42529/76 and 17216/75.

The one or more light-sensitive silver halides used in the photothermographic materials of the present invention are 30 preferably present in an amount of from about 0.005 to about 0.5 mole, more preferably from about 0.01 to about 0.25 mole per mole, and most preferably from about 0.03 to about 0.15 mole, per mole of non-photosensitive source of reducible silver ions.

#### 35 Chemical Sensitizers

The advantages of this invention are provided by chemically sensitizing the silver halide(s) with one or more gold(III)-containing compounds (defined below) in combination with one or more sulfur- or tellurium-containing 40 compounds. The molar ratio of the one or more sulfur- or tellurium-containing compounds to the one or more gold (III)-containing compounds is generally from about 10,000:1 to about 1:10, and preferably from about 5,000:1 to about 1:1.

The total amount of such sulfur- or tellurium-containing 45 compounds in the material will generally vary depending upon the average size of silver halide grains. The silver halide grains are chemically sensitized with these compounds in a total amount generally of at least  $10^{-8}$  mole and preferably from about  $10^{-7}$  to about  $10^{-2}$  mole of sulfur- or tellurium-containing compound per mole of total silver for silver halide grains having an average size of from about 0.01 to about 2  $\mu\text{m}$ .

The total amount of such gold(III)-containing compounds 50 in the material will also generally vary depending upon the average size of silver halide grains with a total amount generally of at least  $10^{-10}$  mole, and preferably from about  $10^{-8}$  to about  $10^{-2}$  mole of gold(III) containing compounds per mole of total silver for silver halide grains having an average size of from about 0.01 to about 2  $\mu\text{m}$ . The upper limit can vary depending upon the compound used, the level of silver halide, and the average grain size, and it would be readily determinable by one of ordinary skill in the art.

A mixture of gold-containing compounds can be used, 55 including a mixture of gold(III)-containing compounds and a mixture of one or more gold(III)-containing compounds and one or more gold(I)-containing compounds. In the latter

mixtures, at least 25 mol % (preferably at least 50 mol %) of the gold-containing compounds are gold(III)-containing compounds defined below in reference to Structure GOLD. Most preferably, all of the gold-containing compounds are in the gold(III) form as defined below.

As long as they provide the desired photospeed increase in the noted combination and do not provide any adverse effects, the gold(III)-containing compounds useful in the practice of this invention are represented by the following Structure GOLD:



## GOLD

wherein L' represents the same or different ligands, each ligand comprising at least one heteroatom that is capable of forming a bond with gold, Y is an anion, r is an integer of from 1 to 8, and q is an integer of from 0 to 3.

More particularly, L' represents the same or different ligands that comprise at least one oxygen, nitrogen, sulfur, or phosphorous atom. Examples of such ligands include but are not limited to, pyridine, bipyridine, terpyridine,

P(phenyl)<sub>3</sub>, carboxylate, imine, phenol, mercaptophenol, imidazole, triazole, and dithiooxamide. The preferred L' ligands are derived from terpyridine, P(phenyl)<sub>3</sub>, and salicylimine compounds.

5 Also in the noted GOLD Structure, Y represents an appropriate counter anion having the appropriate charge. Useful anions include but are not limited to, halides (such as chloride and bromide), perchlorate, tetrafluoroborate, sulfate, sulfonate, methylsulfonate, p-toluenesulfonate, 10 tetrafluoroantimonate, and nitrate. Halides are preferred.

The GOLD Structure also comprises r that is an integer from 1 to 8 (preferably from 1 to 3), and q is 0 or an integer from 1 to 3 (preferably, 3).

Useful gold(III)-containing chemical sensitizers can be 15 prepared using known methods. Representative synthetic methods are described in the literature citations provided in TABLE I above. In addition, some gold(III)-containing compounds can be obtained from various commercial sources including Alfa Aesar (Ward Hill, Mass.).

20 Particularly useful gold(III)-containing chemical sensitizers useful in the practice of this invention are the following Compounds Au-1 to Au-14 shown in TABLE I.

TABLE I

| Compound | Au(III) Complex                     | Ligand-H (L'-H)                                                                      | Method of Preparation                                       |
|----------|-------------------------------------|--------------------------------------------------------------------------------------|-------------------------------------------------------------|
| Au-1     | $\text{AuL}'\text{ClBr}_2$          | P(phenyl) <sub>3</sub>                                                               | F. Mann et al., J. Chem. Soc., 1940, 1235,                  |
| Au-2     | $\text{AuL}'\text{Cl}_3$            |  | L. Hollis et al., J. Am. Chem. Soc., 1983, 105, 4293        |
| Au-3     | $\text{AuL}'\text{Br}_2$            |  | A. Dar et al., J. Chem. Soc., Dalton Trans., 1992, 1907     |
| Au-4     | $\text{AuL}'\text{Cl}_3$            |  | Y. Fuchita et al., J. Chem. Soc., Dalton Trans., 1999, 4431 |
| Au-5     | $\text{L}'[\text{AuP(phenyl)}_2]_3$ |  | W. Hunks et al., Inorg. Chem., 1999, 38, 5930               |
| Au-6     | $\text{AuL}'\text{Cl}_3$            |  | M. Cinelli et al., J. Chem. Soc., Dalton Trans., 1998, 1735 |
| Au-7     | $\text{AuH(L')}_2\text{Cl}_2$       |  | B. Slootmaekers et al., Spectrochim. Acta, 1996, 52A, 1255  |

TABLE I-continued

| Compound | Au(III) Complex                          | Ligand-H (L'—H)             | Method of Preparation                                                                       |
|----------|------------------------------------------|-----------------------------|---------------------------------------------------------------------------------------------|
| Au-8     | $\text{AuL}'\text{Cl}_2$                 |                             | A. Dar et al. J. Chem. Soc., Dalton Trans., 1992, 1907                                      |
| Au-9     | $\text{Au}_2\text{Zn}(\text{L}')_8$      |                             | P. G. Jones et al., Acta Cryst., 1988, C44 1196.                                            |
| Au-10    | $\text{AuPF}_6(\text{L}')_2$             |                             | M. A. Mansour, R. J. Lachicotte, H. J. Gysling, R. Eisenberg, Inorg. Chem., 37 (1998) 4625. |
| Au-11    | $\text{Au}(\text{L}')_2\text{Br}$        |                             | D. J. Radanovic et al., Trans. Met. Chem., 1996, 21, 169                                    |
| Au-12    | $\text{AuL}'\text{Cl}_3$                 |                             | H. G. Raubenheimer et al., Polyhedron, 1992, 11, 893.                                       |
| Au-13    | $\text{Au}(\text{L}')_2(\text{ClO}_4)_3$ | Diferrocenylphenylphosphine | C. M. Gimeno, et al. J. Organomet. Chem., 1999, 579, 206.                                   |
| Au-14    | $\text{AuL}'\text{Cl}$                   | Glycylglycyl-L-histidine    | S. L. Sabine et al., J. Chem. Soc., Dalton Trans., 1997, 2587                               |

As noted above, one or more gold(III)-containing compounds described herein are used in combination with one or more sulfur- or tellurium-containing compounds, all as chemical sensitizers. The one or more gold(III)-containing compounds can also be used in combination with one or more sulfur- and one or more tellurium-containing compounds, all as chemical sensitizers.

Useful tellurium-containing chemical sensitizing compounds are also known in the art, including those described for example, in U.S. Pat. No. 4,639,414 (Sakaguchi et al.), U.S. Pat. No. 6,025,122 (Sakai et al.), U.S. Pat. No. 5,968,725 (Katoh et al.), and *Research Disclosure* Vol. 166, pp. 54-56, 1978.

Particularly useful tellurium-containing compounds are described and claimed in copending and commonly assigned U.S. Ser. No. 09/746,400 (Docket 80836/JLT, noted above). In general, these compounds can be represented by the following Structure I, II, or III.

In Structure I, X represents a COR, CSR, CN(R)<sub>2</sub>, CR, P(R)<sub>2</sub> or P(OR)<sub>2</sub> group that is attached to the two sulfur atoms through the noted carbon or phosphorus atom in the groups. Preferably, X represents a COR, CSR, CN(R)<sub>2</sub>, P(R)<sub>2</sub>, or P(OR)<sub>2</sub> group, and more preferably X is a CN(R)<sub>2</sub> group.

The "R" groups used to define "X" can be any suitable substituted or unsubstituted alkyl group having 1 to 20 carbon atoms (including all possible isomers, such as

45 methyl, ethyl, isopropyl, t-butyl, decyl, trimethylsilylmethyl, and 3-trimethylsilyl-n-propyl), substituted or unsubstituted alkenyl group having 2 to 20 carbon atoms (including all possible isomers such as ethenyl, 1-propenyl, and 2-propenyl) or substituted or unsubstituted carbocyclic or heterocyclic aryl group (Ar) having 6 to 10 carbon atoms in the single- or fused-ring system [such as phenyl, 4-methylphenyl, anthryl, naphthyl, p-methoxyphenyl, 3,5-dimethylphenyl, p-tolyl, mesityl, pyridyl, xylyl, indenyl, 50 2,4,6-tri(t-butyl)-phenyl, pentafluorophenyl, p-methoxyphenyl and 2-phenylethyl]. Preferably, R is a substituted or unsubstituted alkyl group having 1 to 8 carbon atoms such as trimethylsilylmethyl, and 3-trimethylsilyl-n-propyl.

55 Also in Structure I, p is 2 or 4, and preferably, it is 2.

In Structure II, L represents the same or different ligand derived from a neutral Lewis base such as ligands derived from thiourea, substituted thiourea, pyridine, and substituted pyridine groups. Preferably, L is a ligand derived from thiourea or a substituted thiourea, and more preferably, it is a ligand derived from a thiourea as defined below in relation to Structure IV, V, or VI.

X<sup>1</sup> represents a halo (such as chloro, bromo, or iodo), OCN, SCN, S<sub>2</sub>CN(R)<sub>2</sub>, S<sub>2</sub>COR, S<sub>2</sub>CSR, S<sub>2</sub>P(OR)<sub>2</sub>, S<sub>2</sub>P(R)<sub>2</sub>, SeCN, TeCN, CN, SR, OR, N<sub>3</sub>, alkyl (as defined above for R), aryl (as defined above for R), or O<sub>2</sub>CR group wherein R is as defined above. Preferably, X<sup>1</sup> represents a halo (such as

**17**

chloro or bromo), SCN, or  $S_2CN(R)_2$  group, and more preferably, it represents a halo group such as chloro or bromo.

Also in Structure II, m is 0, 1, 2, or 4, and n is 2 and 4 provided that when m is 0 or 2, n is 2 or 4. However, when 5 m is 0 or 2, n is 2 or 4, and when m is 1 or 4, n is 2. Preferably, m is 2 and n is 2 or 4.

In Structure m,  $X^2$  represents a halo, OCN, SCN,  $S_2CN(R)_2$ ,  $S_2COR$ ,  $S_2CSR$ ,  $S_2P(OR)_2$ ,  $S_2P(R)_2$ , SeCN, TeCN, CN, SR, OR,  $N_3$ , alkyl (as defined above for R), aryl (as defined above for Ar), or  $O_2CR$  group (in which R is as defined above). Preferably,  $X^2$  represents a halo, SCN, or SeCN group. More preferably,  $X^2$  is a chloro, bromo, or SCN group.

In addition, R' represents a substituted or unsubstituted alkyl or aryl group that is defined as described above for R. Preferably, R' is a substituted or unsubstituted alkyl groups having from 1 to 10 carbon atoms.

Particularly useful tellurium-containing chemical sensitizers represented by Structures I-III are as follows:



Te-I-1



Te-I-2



Te-I-3



Te-I-4



Te-I-5



Te-I-6



Te-I-7



Te-I-8



Te-I-9



Te-I-10

**18**

-continued

Te-I-11



Te-I-12



Te-I-13



Te-I-14



Te-II-1



Te-II-2



Te-II-3



Te-II-4





Te(S<sub>2</sub>C-phenyl)<sub>2</sub>Te(S<sub>2</sub>CS-*i*-propyl)<sub>2</sub>TeBr<sub>4</sub>(pyridine)<sub>2</sub>

The tellurium-containing chemical sensitizers useful in the present invention can be prepared using readily available starting materials and known procedures as described for example in K. J. Irgolic "The Organic Chemistry of Tellurium", Gordon and Breach, N.Y., 1974, K. J. Irgolic, "Houben Weyl Methods of Organic Chemistry", Vol. E 12b, "Organotellurium Compounds", D. Klamann, Ed., Georg Thieme Verlag, Stuttgart, Germany, 1990, *Synthetic Method of Organometallic and Inorganic Chemistry*, W. A. Herrmann and C. Zybill, Eds., George Thieme Verlag, N.Y., 1997; Vol. 4, Chapter 3: K. J. Irgolic, Tellurium and its Compounds, *The Chemistry of Organic Selenium and Tellurium Compounds*, Vol. 1 (1986) and Vol. 2 (1987), S. Patai and Z. Rappoport, Eds., Wiley, New York, H. J. Gysling, H. R. Luss, and D. L. Smith, *Inorg. Chem.*, 1979, 18, 2696 and H. J. Gysling, M. Lelemental, M. G. Mason, and L. J. Gerenser, *J. Phot. Sci.*, 1982, 30, 55. Compound II-1, [TeCl<sub>4</sub>(tetramethylthiourea)<sub>2</sub>], was prepared as described in O. Foss and W. Johannessen, *Acta Chem. Scand.*, 1961, 15, 1939. A representative synthesis of Compound Te-I-1 is provided in U.S. Ser. No. 09/746,400 (Docket 80836/JLT, noted above).

Sulfur-containing chemical sensitizers useful in the present invention are well known in the art and described for example, in Sheppard et al., *J. Franklin Inst.*, 1923, 196, pp. 653 and 673, C. E. K. Mees and T. H. James, *The Theory of the Photographic Process*, 4<sup>th</sup> Edition, 1977, pp. 152-3, Tani, T., *Photographic Sensitivity: Theory and Mechanisms*, Oxford University Press, N.Y., 1995, pp. 167-176, U.S. Pat. No. 5,891,615 (Winslow et al.), Zavlin et al., IS&T's 48<sup>th</sup> Annual Conference Papers, May 7-11 1995 Washington D.C., pp. 156-6), U.S. Pat. No. 4,810,626 (Burgmaier et al.), U.S. Pat. No. 4,036,650 (Kobayashi et al.), U.S. Pat. No. 4,213,784 (Ikenoue et al.), and U.S. Pat. No. 4,207,108 (Hiller).

Particularly useful sulfur-containing chemical sensitizers are substituted thiourea ligands that include any  $-\text{S}=\text{C}(-\text{N}<\text{N}<-\text{N})-$  group that has one or more of the four nitrogen valences substituted with hydrogen or with the same or different aliphatic substituents. More preferably, the four nitrogen valences are substituted with the same aliphatic substituent.

Useful thioureas are described in U.S. Ser. No. 09/667, 748 (noted above) and in U.S. Pat. No. 5,843,632 (Eshelman et al.), both incorporated herein by reference. In general, these compounds can be represented by below by Structure IV, V, or VI:



-continued

Te-III-6

Te-III-7

Te-III-8

5



In Structure IV, R<sub>1</sub>, R<sub>2</sub>, R<sub>3</sub>, and R<sub>4</sub> independently represent hydrogen, substituted or unsubstituted alkyl groups (including alkylenearyl groups such as benzyl), substituted or unsubstituted aryl groups (including arylenealkyl groups), substituted or unsubstituted cycloalkyl groups, substituted or unsubstituted alkenyl groups, substituted or unsubstituted alkynyl groups and heterocyclic groups.

Useful alkyl groups are branched or linear and can have from 1 to 20 carbon atoms (preferably having 1 to 5 carbon atoms), useful aryl groups can have from 6 to 14 carbon atoms in the carbocyclic ring, useful cycloalkyl groups can have from 5 to 14 carbon atoms in the central ring system, useful alkenyl and alkynyl groups can be branched or linear and have from 2 to 20 carbon atoms, and useful heterocyclic groups can have 5 to 10 carbon, oxygen, sulfur and nitrogen atoms in the central ring system (they can also have fused rings).

These various monovalent groups can be further substituted with one or more groups including but not limited to, halo groups, alkoxy carbonyl groups, hydroxy groups, alkoxy groups, cyano groups, acyl groups, acyloxy groups, carbonyloxy ester groups, sulfonic acid ester groups, alkylthio groups, dialkylamino groups, carboxylic acid groups, sulfonic acid groups, hydroxylamino groups, sulfo groups, phosphono groups, and any other group readily apparent to one skilled in the art. R<sub>1</sub>, R<sub>2</sub>, R<sub>3</sub>, R<sub>4</sub> and R<sub>5</sub> can independently be alkyl groups.

Alternatively, R<sub>1</sub> and R<sub>3</sub> taken together, R<sub>2</sub> and R<sub>4</sub> taken together, R<sub>1</sub> and R<sub>2</sub> taken together, or R<sub>3</sub> and R<sub>4</sub> taken together, can form a substituted or unsubstituted 5- to 7-membered heterocyclic ring.

Where R<sub>1</sub> and R<sub>3</sub> are taken together or R<sub>2</sub> and R<sub>4</sub> are taken together, the heterocyclic rings can be saturated or unsaturated and can contain oxygen, nitrogen or sulfur atoms in addition to carbon atoms. Useful rings of this type include, but are not limited to, imidazole, pyrrolidine, pyrrolidine, thiohydantoin, pyridone, morpholine, piperazine and thiomorpholine rings. These rings can be substituted with one or more alkyl groups (having 1 to 5 carbon atoms), aryl groups (having 6 to 10 carbon atoms in the central ring system), cycloalkyl groups (having 5 to 10 carbon atoms in the central ring system), alkoxy groups, carbonyloxy ester groups, halo groups, cyano groups, hydroxy groups, acyl groups, alkoxy carbonyl groups, sulfonic ester groups, alkylthio groups, carbonyl groups, carboxylic acid groups, sulfonic acid groups, hydroxylamino groups, sulfo groups, phosphono groups, and other groups readily apparent to one skilled in the art.

Where R<sub>1</sub> and R<sub>2</sub> are taken together or R<sub>3</sub> and R<sub>4</sub> are taken together, the heterocyclic rings can be saturated or unsaturated and can contain oxygen, nitrogen or sulfur atoms in addition to carbon atoms. Useful rings of this type include, but are not limited to, 2-imidazolidine-thione, 2-thioxo-1-imidazolidinone (thiohydantoin), 1,3-dihydro-2H-imidazole-2-thione, 1,3-dihydro-2H-benzimidazole-2-thione, tetrahydro-2,2-thioxo-5-pyrimidine, tetrahydro-1,3,5-triazine-2(1H)-thione, dihydro-2-thioxo-4,6-(1H,3H)-pyrimidinedione, dihydro-1,3,5-triazine-2,4-(1H,3H)-dione and hexahydro-diazepine-2-thione rings. These rings can be

substituted with one or more alkyl groups (having 1 to 5 carbon atoms), aryl groups (having 6 to 10 carbon atoms in the central ring system), cycloalkyl groups (having 5 to 10 carbon atoms in the central ring system), carboxyloxyester groups, halo groups, cyano groups, hydroxy groups, acyl groups, alkoxycarbonyl groups, sulfonic ester groups, alkylthio groups, carbonyl groups, alkoxy groups carboxylic acid groups, sulfonic acid groups, hydroxylamino groups, sulfo groups, phosphono groups, and other groups readily apparent to one skilled in the art.

Preferably,  $R_1$ ,  $R_2$ ,  $R_3$ , and  $R_4$  independently represent alkyl, alkenyl, alkynyl, aryl, and heterocyclic groups, more preferably alkyl, aryl, and alkenyl groups, and most preferably alkenyl groups. A preferred alkenyl group is an allyl group. A preferred alkyl group is a methyl group. Also particularly useful are sulfur-containing 1,1,3,3-tetrasubstituted thiourea compounds having carboxylic acid groups, sulfonic acid groups, or other acid groups that have an acid dissociation constant (pKa) of less than 7.

In Structure V noted above,  $R_1$ ,  $R_2$ ,  $R_3$ ,  $R_4$  and  $R_5$  have the same definitions as noted above for  $R_1$ ,  $R_2$ ,  $R_3$  and  $R_4$  in Structure I with the following differences:

$R_1$  and  $R_3$  can be taken together,  $R_2$  and  $R_4$  can be taken together,  $R_3$  and  $R_5$  can be taken together and/or  $R_4$  and  $R_5$  can be taken together, to form substituted or unsubstituted 5- to 7-membered heterocyclic rings (as described above for Structure IV). When those heterocyclic rings are formed from  $R_1$  and  $R_3$  taken together or  $R_2$  and  $R_4$  taken together, they are as defined above for  $R_1$  and  $R_3$  taken together for Structure I, but the resulting heterocyclic rings can have other substituents such as alkoxy groups, dialkylamino groups, and carboxylic acid groups, sulfonic acid groups, hydroxylamino groups, sulfo, phosphono and other acidic groups. When those heterocyclic rings are formed from  $R_3$  and  $R_5$  taken together or  $R_4$  and  $R_5$  taken together, they can be substituted as described for  $R_1$  and  $R_3$  of Structure IV. Useful rings of this type include, but are not limited to, 2-imidazolidinethione, 2-thioxo-1-imidazolidinone (thiohydantoin), 1,3-dihydro-2H-imidazole-2-thione, 1,3-dihydro-2H-benzimidazole-2-thione, tetrahydro-2,2-thioxo-5-pyrimidine, tetrahydro-1,3,5-triazine-2(1H)-thione, dihydro-2-thioxo-4,6-(1H, 3H)-pyrimidinedione, dihydro-1,3,5-triazine-2,4-(1H, 3H)-dione and hexahydro diazepine-2-thione.

For Structure V, the preferred groups for  $R_1$ – $R_5$  are hydrogen, alkyl, alkenyl, alkynyl, aryl, and heterocyclic groups, more preferably alkyl, aryl, and alkenyl groups, and more preferably alkenyl groups. A preferred alkenyl group is an allyl group.

Also, in Structure V, most preferable alkyl groups are methyl and ethyl groups. Most preferable aryl groups are phenyl or tolyl groups. Most preferable cycloalkyl groups are cyclopentyl and cyclohexyl groups. Most preferably the alkenyl group is an allyl group. Most preferable heterocyclic groups are morpholino and piperazino groups.

In Structure VI noted above,  $R_1$ ,  $R_2$ ,  $R_3$ ,  $R_4$ ,  $R_5$ , and  $R_6$  have the same definitions as noted above for  $R_1$ ,  $R_2$ ,  $R_3$ ,  $R_4$ , and  $R_5$  in Structure V described above. In addition,  $R_3$  and  $R_6$  taken together,  $R_4$  and  $R_5$  taken together,  $R_1$  and  $R_3$  taken together,  $R_2$  and  $R_4$  taken together, or  $R_5$  and  $R_6$  taken together, can form a substituted or unsubstituted 5- to 7-membered heterocyclic ring as described above for the heterocyclic rings in Structure V.

$R_7$  is a divalent aliphatic or alicyclic linking group including but not limited to substituted or unsubstituted alkylene groups having 1 to 12 carbon atoms, substituted or unsubstituted cycloalkylene groups having 5 to 8 carbon

atoms in the ring structure, substituted or unsubstituted arylene groups having 6 to 10 carbon atoms in the ring structure, substituted or unsubstituted divalent heterocycl groups having 5 to 10 carbon, nitrogen, oxygen, and sulfur atoms in the ring structure, or any combination of two or more of these divalent groups, or any two or more of these groups connected by ether, thioether, carbonyl, carbonamido, sulfoamido, amino, imido, thiocarbonyl, thioamido, sulfinyl, sulfonyl, or phosphinyl groups. Preferably,  $R_7$  is a substituted or unsubstituted alkylene group having at least 2 carbon atoms.

Representative examples of compounds represented by Structures IV—VI are as follows:

S-IV-1



S-IV-2



S-IV-3



S-IV-4



S-IV-5



S-IV-6



S-IV-7



25

-continued



26

-continued

S-IV-16



27

-continued



28

-continued

S-IV-34



**29**

-continued

**30**

-continued



31

-continued



Another class of sulfur-containing chemical sensitizers particularly useful with the gold(III)-containing compounds

32

described herein, are compounds with sulfur atoms directly attached to cyclic rings within the structure, particularly dye structures, more preferably with at least some sulfur atoms attached or incorporated as thiocarbonyl groups (that is,  $>\text{C}=\text{S}$ ) or as  $-\text{S}-$  groups within the actual ring structure of the compounds. Compounds with both types of sulfur atom positioning [that is, both  $>\text{C}=\text{S}$  and  $-\text{S}-$ , or  $-\text{S}-(\text{C}=\text{S})-$ ] are also desirable in the practice of the present invention. In some instances, the sulfur-containing compound is an organic sulfur-containing compound that is also known in the art as a spectral sensitizing dye. Such compounds are described for example in U.S. Pat. No. 5,891,615 (Winslow et al.), incorporated herein by reference. Upon decomposition in an oxidizing environment, such compounds provide chemical sensitization instead of spectral sensitization. In such embodiments, the method of preparing photothermographic emulsions will likely further comprise adding a second spectral sensitizing dye to the photothermographic emulsion to spectrally sensitize the silver halide grains.

Preferred sulfur containing chemical sensitizing compounds of this type contain the thiohydantoin, rhodanine, or the 2-thio-4-oxo-oxazolidine nucleus. These nuclei are shown below. In general, these nuclei can be represented below by Structure VII, VIII, or IX:



VII



VIII



IX

Representative sulfur containing chemical sensitizing compounds useful in the present invention and their methods 55 of preparation and sources are known in the art. These representations are exemplary and are not intended to be limiting.



S-VII-1

33

-continued



34

-continued

S-VII-2



S-VIII-7

5



S-VIII-1 15



S-VIII-8

20



S-VIII-2 25



S-VIII-9

30



S-VIII-3



S-IX-1

35



S-VIII-4

Useful sulfur-containing chemical sensitizers can be purchased from a number of commercial sources (such as 40 Aldrich Chemical Co.), or prepared using readily available starting materials and known procedures as described for example in Belgian Patent Publication 813,926 (May 27, 1959), Schroeder, *Chem. Rev.* 1955, pp. 181-228, Barluenga et al., *Comprehensive Organic Functional Group Transformations*, Vol. 6, 1995, (Kratzky et al., Eds.), pp. 569-585 and references cited therein, and Karkhanis et al., *Phosphorous and Sulfur*, 1985, 22, pp. 49-57. A representative synthesis of Compound S-IV-2 is provided in U.S. Ser. No. 09/667,748 (noted above).

50 Additional and conventional chemical sensitizers may be used in combination with the combination of chemical sensitizing compounds described above. Such compounds may contain gold(I), selenium, platinum, palladium, 55 ruthenium, rhodium, iridium, or combinations thereof, a reducing agent such as a tin halide or a combination of any of these. The details of these materials are provided for example in T. H. James, *The Theory of the Photographic Process*, Fourth Edition, Chapter 5, pp. 149-169. Suitable



S-VIII-5

60 conventional chemical sensitization procedures are also described in U.S. Pat. No. 1,623,499 (Sheppard et al.), U.S. Pat. No. 2,399,083 (Waller et al.), U.S. Pat. No. 3,297,447 (McVeigh), U.S. Pat. No. 3,297,446 (Dunn), U.S. Pat. No. 5,049,485 (Deaton), U.S. Pat. No. 5,252,455 (Deaton), U.S. Pat. No. 5,391,727 (Deaton), U.S. Pat. No. 5,912,111 (Lok et al.), U.S. Pat. No. 5,759,761 (Lushington et al.), and EP-A-0 915 371 (Lok et al.).



S-VIII-6

65

In some embodiments of the present invention, the photothermographic materials comprise a merocyanine spectral sensitizing dye and the photosensitive silver halide has been chemically sensitized with a tellurium-containing compound in combination with said gold(III)-containing compound.

As noted above, the photothermographic emulsions useful to make the imaging materials of this invention can be prepared by:

- A) providing a photothermographic emulsion comprising photosensitive silver halide grains and a non-photosensitive source of reducible silver ions, and
- B) positioning one or more of the defined gold(III)-containing and sulfur- or tellurium-containing chemical sensitizers on or around the photosensitive silver halide grains.

More particularly, such a method can comprise:

- A) providing photosensitive silver halide grains,
- B) providing a photothermographic emulsion of the photosensitive silver halide grains and a non-photosensitive source of reducible silver ions, and
- C) prior to, during or immediately following either or both of steps A and B, chemically sensitizing the photosensitive silver halide grains with the defined gold(III)-containing and sulfur- or tellurium-containing chemical sensitizers described above.

The chemical sensitizers described herein can be added at one or more times and at any stage of preparation of the photothermographic emulsion formulations.

In some embodiments of the method of preparing photothermographic emulsions, step C can follow step B. That is, chemical sensitization can take place after the formation of the non-photosensitive source of reducible silver in the presence of the preformed silver halide grains or the mixing of the non-photosensitive source of reducible silver in the presence of the preformed photosensitive silver halide grains (that is, during the formation of the silver soap). Chemical sensitization can also take place at any stage during the formulation of the photothermographic emulsion, such as during or after addition of pyridinium hydrobromide perbromide, calcium bromide, zinc bromide or similar addenda, before any toning agents (described below) are added to the formulation, or before any spectral sensitizing dyes (described below) are added. The silver halide grains may even be chemically sensitized as the last step in the formation of the photothermographic emulsion.

Alternatively, step C can be carried out between steps A and B. In this instance, the preformed photosensitive silver halide grains are chemically sensitized immediately before they are mixed with the non-photosensitive source of reducible silver ions, or immediately before the non-photosensitive source of reducible silver ions is formed in their presence.

Still further, step C can be carried out prior to step A by chemically sensitizing preformed photosensitive silver halide grains during or immediately after their preparation and before they are mixed with the non-photosensitive source of reducible silver ions or before the non-photosensitive source of reducible silver ions is reduced in their presence.

When the photosensitive silver halide grains are chemically sensitized with an organic sulfur-containing compound containing a thiohydantoin, rhodanine, or 2-thio-4-oxo-oxazolidine nucleus, step C also includes decomposing the sulfur-containing compound on or around the photosensitive silver halide grains in an oxidizing environment.

The chemical sensitizers described herein can be present in one or more imaging layer(s) on the front side of the

photothermographic material. Preferably, they are used on all photosensitive silver halide grains within the material.

It would be readily determinable by routine experimentation as to the optimum time for adding particular chemical sensitizers to achieve the maximum speed enhancement in the photothermographic emulsion.

To further control the properties of photothermographic materials, (for example, contrast,  $D_{min}$ , speed, or fog), it may be preferable to add one or more heteroaromatic mercapto compounds or heteroaromatic disulfide compounds of the formulae:  $Ar-S-M$  and  $Ar-S-S-Ar$ , wherein M represents a hydrogen atom or an alkali metal atom and Ar represents a heteroaromatic ring or fused heteroaromatic ring containing one or more of nitrogen, sulfur, oxygen, selenium, or tellurium atoms. Preferably, the heteroaromatic ring comprises benzimidazole, naphthimidazole, benzothiazole, naphthothiazole, benzoxazole, naphthoxazole, benzoselenazole, benzotellurazole, imidazole, oxazole, pyrazole, triazole, thiazole, thiadiazole, tetrazole, triazine, pyrimidine, pyridazine, pyrazine, pyridine, purine, quinoline, or quinazolinone. Compounds having other heteroaromatic rings are also envisioned to be suitable. For example, heteroaromatic mercapto compounds are described as supersensitizers for infrared photothermographic materials in EP-A-0 559 228. (Philip Jr. et al.).

The heteroaromatic ring may also carry substituents. Examples of preferred substituents are halo groups (such as bromo and chloro), hydroxy, amino, carboxy, alkyl groups (for example, of 1 or more carbon atoms and preferably 1 to 4 carbon atoms), and alkoxy groups (for example, of 1 or more carbon atoms and preferably of 1 to 4 carbon atoms).

Heteroaromatic mercapto compounds are most preferred. Examples of preferred heteroaromatic mercapto compounds are 2-mercaptopbenzimidazole, 2-mercaptop-5-methylbenzimidazole, 2-mercaptopbenzothiazole, and 2-mercaptopbenzoxazole. Mixtures of such compounds can also be used.

If used, a heteroaromatic mercapto compound is generally present in an emulsion layer in an amount of at least about 0.0001 mole per mole of total silver in the emulsion layer. More preferably, the heteroaromatic mercapto compound is present within a range of about 0.001 mole to about 1.0 mole, and most preferably, about 0.005 mole to about 0.2 mole, per mole of total silver.

#### Spectral Sensitizing Compounds

It may also be desirable to add spectral sensitizing dyes to enhance silver halide sensitivity to ultraviolet, visible and infrared light. Thus, the photosensitive silver halides may be spectrally sensitized with various dyes that are known to spectrally sensitize silver halide. Non-limiting examples of spectral sensitizing dyes that can be employed include cyanine dyes, merocyanine dyes, complex cyanine dyes, complex merocyanine dyes, holopolar cyanine dyes, hemicyanine dyes, styryl dyes, and hemioxanol dyes. The cyanine dyes, merocyanine dyes and complex merocyanine dyes are particularly useful. Suitable spectral sensitizing dyes such as those described in U.S. Pat. No. 3,719,495 (Lea), U.S. Pat. No. 5,393,654 (Burrows et al.), U.S. Pat. No. 5,441,866 (Miller et al.) and U.S. Pat. No. 5,281,515 (Delprato et al.) and U.S. Pat. No. 5,314,795 (Helland et al.) are effective in the practice of the invention.

These spectral sensitizing dyes can be used in addition to the organic sulfur-containing compounds described above that are used to chemically sensitize photosensitive silver halide grains in an oxidative environment.

An appropriate amount of sensitizing dye added is generally about  $10^{-10}$  to  $10^{-1}$  mole, and preferably, about  $10^{-7}$  to  $10^{-2}$  moles per mole of silver halide.

## Non-Photosensitive Source of Reducible Silver Ions

The non-photosensitive source of reducible silver ions used in photothermographic materials of this invention can be any compound that contains reducible silver (1+) ions. Preferably, it is a silver salt that is comparatively stable to light and forms a silver image when heated to 50° C. or higher in the presence of an exposed photocatalyst (such as silver halide) and a reducing composition.

Silver salts of organic acids, particularly silver salts of long-chain carboxylic acids are preferred. The chains typically contain 10 to 30, and preferably 15 to 28, carbon atoms. Suitable organic silver salts include silver salts of organic compounds having a carboxylic acid group. Examples thereof include a silver salt of an aliphatic carboxylic acid or a silver salt of an aromatic carboxylic acid. Preferred examples of the silver salts of aliphatic carboxylic acids include silver behenate, silver arachidate, silver stearate, silver oleate, silver laurate, silver caprate, silver myristate, silver palmitate, silver maleate, silver fumarate, silver tartarate, silver furoate, silver linoleate, silver butyrate, silver camphorate, and mixtures thereof. Preferred examples of the silver salts of aromatic carboxylic acid and other carboxylic acid group-containing compounds include, but are not limited to, silver benzoates, a silver-substituted benzoate, such as silver 3,5-dihydroxy-benzoate, silver o-methylbenzoate, silver m-methylbenzoate, silver p-methylbenzoate, silver 2,4-dichlorobenzoate, silver acetamidobenzoate, silver p-phenylbenzoate, silver gallate, silver tannate, silver phthalate, silver terephthalate, silver salicylate, silver phenylacetate, silver pyromellitate, a silver salt of 3-carboxymethyl-4-methyl-4-thiazoline-2-thione or others as described in U.S. Pat. No. 3,785,830 (Sullivan et al.), and silver salts of aliphatic carboxylic acids containing a thioether group as described in U.S. Pat. No. 3,330,663 (Weyde et al.). Soluble silver carboxylates comprising hydrocarbon chains incorporating ether or thioether linkages, or sterically hindered substitution in the  $\alpha$ - (on a hydrocarbon group) or ortho- (on an aromatic group) position, and displaying increased solubility in coating solvents and affording coatings with less light scattering can also be used. Such silver carboxylates are described in U.S. Pat. No. 5,491,059 (Whitcomb). Mixtures of any of the silver salts described herein can also be used if desired.

Silver salts of sulfonates are also useful in the practice of this invention. Such materials are described for example in U.S. Pat. No. 4,504,575 (Lee). Silver salts of sulfosuccinates are also useful as described for example in EP-A-0 227 141 (Leenders et al.).

Silver salts of compounds containing mercapto or thione groups and derivatives thereof can also be used. Preferred examples of these compounds include, but are not limited to, a silver salt of 3-mercaptop-4-phenyl-1,2,4-triazole, a silver salt of 2-mercaptopbenzimidazole, a silver salt of 2-mercaptop-5-amino-thiadiazole, a silver salt of 2-(2-ethylglycolamido)benzothiazole, silver salts of thioglycolic acids (such as a silver salt of a S-alkylthioglycolic acid, wherein the alkyl group has from 12 to 22 carbon atoms), silver salts of dithiocarboxylic acids (such as a silver salt of dithioacetic acid), a silver salt of thioamide, a silver salt of 5-carboxylic-1-methyl-2-phenyl-4-thiopyridine, a silver salt of mercaptotriazine, a silver salt of 2-mercaptopbenzoxazole, silver salts as described in U.S. Pat. No. 4,123,274 (Knight et al.) (for example, a silver salt of a 1,2,4-mercaptopthiazole derivative, such as a silver salt of 3-amino-5-benzylthio-1,2,4-thiazole), and a silver salt of thione compounds [such as a silver salt of 3-(2-carboxyethyl)-4-methyl-4-thiazoline-2-thione as described in U.S. Pat. No. 3,201,678 (Meixell)].

Furthermore, a silver salt of a compound containing an imino group can be used. Preferred examples of these compounds include, but are not limited to, silver salts of benzotriazole and substituted derivatives thereof (for example, silver methylbenzotriazole and silver 5-chlorobenzotriazole), silver salts of 1,2,4-triazoles or 1-H-tetrazoles such as phenylmercaptotetrazole as described in U.S. Pat. No. 4,220,709 (deMauriac), and silver salts of imidazoles and imidazole derivatives as described in U.S. Pat. No. 4,260,677 (Winslow et al.). Moreover, silver salts of acetylenes can also be used as described, for example in U.S. Pat. No. 4,761,361 (Ozaki et al.) and U.S. Pat. No. 4,775,613 (Hirai et al.).

It is also convenient to use silver half soaps. A preferred example of a silver half soap is an equimolar blend of silver carboxylate and carboxylic acid, which analyzes for about 14.5% by weight solids of silver in the blend and which is prepared by precipitation from an aqueous solution of the sodium salt of a commercial fatty carboxylic acid, or by addition of the free fatty acid to the silver soap. For transparent films a silver carboxylate full soap, containing not more than about 15% of free carboxylic acid and analyzing for about 22% silver, can be used. For opaque photothermographic materials, different amounts can be used.

The methods used for making silver soap emulsions are well known in the art and are disclosed in *Research Disclosure*, April 1983, item 22812, *Research Disclosure*, October 1983, item 23419, U.S. Pat. No. 3,985,565 (Gabrielsen et al.) and the references cited above.

The photocatalyst and the non-photosensitive source of reducible silver ions must be in catalytic proximity (that is, reactive association). "Catalytic proximity" or "reactive association" means that they should be in the same layer, or in adjacent layers. It is preferred that these reactive components be present in the same emulsion layer.

The one or more non-photosensitive sources of reducible silver ions are preferably present in an amount of about 5% by weight to about 70% by weight, and more preferably, about 10% to about 50% by weight, based on the total dry weight of the emulsion layers. Stated another way, the amount of the sources of reducible silver ions is generally present in an amount of from about 0.001 to about 0.2 mol/m<sup>2</sup> of the dry photothermographic material, and preferably from about 0.01 to about 0.05 mol/m<sup>2</sup> of that material.

The total amount of silver (from all silver sources) in the photothermographic materials is generally at least 0.002 mol/m<sup>2</sup> and preferably from about 0.01 to about 0.05 mol/m<sup>2</sup>.

## Reducing Agents

The reducing agent (or reducing agent composition comprising two or more components) for the source of reducible silver ions can be any material, preferably an organic material, that can reduce silver (I) ion to metallic silver. Conventional photographic developers such as methyl gallate, hydroquinone, substituted hydroquinones, hindered phenols, amidoximes, azines, catechol, pyrogallol, ascorbic acid (and derivatives thereof), leuco dyes and other materials readily apparent to one skilled in the art can be used in this manner as described for example in U.S. Pat. No. 6,020,117 (Bauer et al.).

In some instances, the reducing agent composition comprises two or more components such as a hindered phenol developer and a co-developer that can be chosen from the various classes of reducing agents described below. Ternary developer mixtures involving the further addition of contrast

enhancing agents are also useful. Such contrast enhancing agents can be chosen from the various classes of reducing agents described below.

Hindered phenol reducing agents are preferred (alone or in combination with one or more co-developers and contrast enhancing agents). These are compounds that contain only one hydroxy group on a given phenyl ring and have at least one additional substituent located ortho to the hydroxy group. Hindered phenol developers may contain more than one hydroxy group as long as each hydroxy group is located on different phenyl rings. Hindered phenol developers include, for example, binaphthols (that is dihydroxybinaphthyls), biphenols (that is dihydroxybiphenyls), bis(hydroxynaphthyl)methanes, bis(hydroxyphenyl)methanes, hindered phenols, and hindered naphthols each of which may be variously substituted.

Representative binaphthols include, but are not limited, to 1,1'-bi-2-naphthol, 1,1'-bi-4-methyl-2-naphthol and 6,6'-dibromo-bi-2-naphthol. For additional compounds see U.S. Pat. No. 3,094,417 (Workman) and U.S. Pat. No. 5,262,295 (Tanaka et al.), both incorporated herein by reference.

Representative biphenols include, but are not limited, to 2,2'-dihydroxy-3,3'-di-t-butyl-5,5-dimethylbiphenyl, 2,2'-dihydroxy-3,3',5,5'-tetra-t-butylbiphenyl, 2,2'-dihydroxy-3,3'-di-t-butyl-5,5'-dichloro-biphenyl, 2-(2-hydroxy-3-t-butyl-5-methylphenyl)-4-methyl-6-n-hexylphenol, 4,4'-dihydroxy-3,3',5,5'-tetra-t-butylbiphenyl and 4,4'-dihydroxy-3,3',5,5'-tetramethylbiphenyl. For additional compounds see U.S. Pat. No. 5,262,295 (noted above).

Representative bis(hydroxynaphthyl)methanes include, but are not limited to, 4,4'-methylenebis(2-methyl-1-naphthol). For additional compounds see U.S. Pat. No. 5,262,295 (noted above).

Representative bis(hydroxyphenyl)methanes include, but are not limited to, bis(2-hydroxy-3-t-butyl-5-methylphenyl) methane (CAO-5), 1,1-bis(2-hydroxy-3,5-dimethylphenyl)-3,5,5-trimethylhexane (NONOX or PERMANAX WSO), 1,1-bis(3,5-di-t-butyl-4-hydroxyphenyl)methane, 2,2-bis(4-hydroxy-3-methylphenyl)propane, 4,4-ethylidene-bis(2-t-butyl-6-methylphenol) and 2,2-bis(3,5-dimethyl-4-hydroxyphenyl)propane. For additional compounds see U.S. Pat. No. 5,262,295 (noted above).

Representative hindered phenols include, but are not limited to, 2,6-di-t-butylphenol, 2,6-di-t-butyl-4-methylphenol, 2,4-di-t-butylphenol, 2,6-dichlorophenol, 2,6-dimethylphenol and 2-t-butyl-6-methylphenol.

Representative hindered naphthols include, but are not limited to, 1-naphthol, 4-methyl-1-naphthol, 4-methoxy-1-naphthol, 4-chloro-1-naphthol and 2-methyl-1-naphthol. For additional compounds see U.S. Pat. No. 5,262,295 (noted above).

More specific alternative reducing agents that have been disclosed in dry silver systems including amidoximes such as phenylamidoxime, 2-thienyl-amidoxime and p-phenoxyphenylamidoxime, azines (for example, 4-hydroxy-3,5-dimethoxybenzaldehydrazine), a combination of aliphatic carboxylic acid aryl hydrazides and ascorbic acid, such as 2,2'-bis(hydroxymethyl)-propionyl- $\beta$ -phenyl hydrazide in combination with ascorbic acid, a combination of polyhydroxy-benzene and hydroxylamine, a reductone and/or a hydrazine [for example, a combination of hydroquinone and bis(ethoxyethyl)hydroxylamine], piperidino-hexose reductone or formyl-4-methylphenylhydrazine, hydroxamic acids (such as phenylhydroxamic acid, p-hydroxyphenylhydroxamic acid, and o-alanine-hydroxamic acid), a combination of azines and sulfonamidophenols (for example, phenothiazine and 2,6-dichloro-4-

benzenesulfonamidophenol),  $\alpha$ -cyanophenyl-acetic acid derivatives (such as ethyl  $\alpha$ -cyano-2-methylphenylacetate and ethyl  $\alpha$ -cyanophenylacetate), bis-o-naphthols [such as 2,2'-dihydroxyl-1-binaphthyl, 6,6'-dibromo-2,2'-dihydroxy-1,1'-binaphthyl, and bis(2-hydroxy-1-naphthyl)-methane], a combination of bis-o-naphthol and a 1,3-dihydroxybenzene derivative (for example, 2,4-dihydroxybenzophenone or 2,4-dihydroxyacetophenone), 5-pyrazolones such as 3-methyl-1-phenyl-5-pyrazolone, reductones (such as dimethylaminohexose reductone, anhydrodihydro-aminohexose reductone and anhydromethoxy-piperidone-hexose reductone), sulfonamidophenol reducing agents (such as 2,6-dichloro-4-benzenesulfonamido-phenol, and p-benzenesulfonamidophenol), 2-phenylindane-1,3-dione and similar compounds, chromans (such as 2,2-dimethyl-7-t-butyl-6-hydroxychroman), 1,4-dihydropyridines (such as 2,6-dimethoxy-3,5-dicarbethoxy-1,4-dihydropyridine), bisphenols [such as bis(2-hydroxy-3-t-butyl-5-methylphenyl)methane, 2,2-bis(4-hydroxy-3-methylphenyl) propane, 4,4-ethylidene-bis(2-t-butyl-6-methylphenol) and 2,2-bis(3,5-dimethyl-4-hydroxyphenyl)propane], ascorbic acid derivatives (such as 1-ascorbylpalmitate, ascorbylstearate and unsaturated aldehydes and ketones), 3-pyrazolidones, and certain indane-1,3-diones.

An additional class of reducing agents that can be used as developers are substituted hydrazines including the sulfonyl hydrazides described in U.S. Pat. No. 5,464,738 (Lynch et al.). Still other useful reducing agents are described, for example, in U.S. Pat. No. 3,074,809 (Owen), U.S. Pat. No. 3,094,417 (Workman), U.S. Pat. No. 3,080,254 (Grant, Jr.) and U.S. Pat. No. 3,887,417 (Klein et al.). Auxiliary reducing agents may be useful as described in U.S. Pat. No. 5,981,151 (Leenders et al.).

Useful co-developer reducing agents can also be used as described for example, in copending U.S. Ser. No. 09/239,182 (filed Jan. 28, 1999 by Lynch and Skoog), incorporated herein by reference. Examples of these compounds include, but are not limited to, 2,5-dioxo-cyclopentane carboxaldehyde, 5-(hydroxymethylene)-2,2-dimethyl-1,3-dioxane-4,6-dione, 5-(hydroxy-methylene)-1,3-dialkylbarbituric acids, 2-(ethoxymethylene)-1H-indene-1,3(2H)-dione.

Additional classes of reducing agents that can be used as co-developers are trityl hydrazides and formyl phenyl hydrazides as described in U.S. Pat. No. 5,496,695 (Simpson et al.), 3-heteroaromatic-substituted acrylonitrile compounds as described in U.S. Pat. No. 5,635,339 (Murray), 2-substituted malondialdehyde compounds as described in U.S. Pat. No. 5,654,130 (Murray), substituted propenitriles as described in U.S. Pat. No. 5,686,228 (Murray et al.), and 4-substituted isoxazole compounds as described in U.S. Pat. No. 5,705,324 (Murray). Still other useful co-developers include 2,5-dioxo-cyclopentane carboxaldehydes, 5-(hydroxymethylene)-1,3-dialkylbarbituric acids, and 2-(ethoxymethylene)-1H-indene-1,3(2H)-diones. Additional developers are described in U.S. Pat. No. 6,100,022 (Inoue et al.).

Various contrast enhancers can be used in some photothermographic materials with specific co-developers. Examples of useful contrast enhancers include, but are not limited to, hydroxylamines (including hydroxylamine and alkyl- and aryl-substituted derivatives thereof), alkanolamines and ammonium phthalamate compounds as described for example, in U.S. Pat. No. 5,545,505 (Simpson), hydroxamic acid compounds as described for example, in U.S. Pat. No. 5,545,507 (Simpson et al.), N-acylhydrazine compounds as described for example, in U.S. Pat. No. 5,558,983

(Simpson et al.), and hydrogen atom donor compounds as described in U.S. Pat. No. 5,637,449 (Harring et al.).

The reducing agent (or mixture thereof) described herein is generally present as 1 to 10% (dry weight) of the emulsion layer. In multilayer constructions, if the reducing agent is added to a layer other than an emulsion layer, slightly higher proportions, of from about 2 to 15 weight % may be more desirable. Any co-developers may be present generally in an amount of from about 0.001% to about 1.5% (dry weight) of the emulsion layer coating.

#### Other Addenda

The photothermographic materials of the invention can also contain other additives such as shelf-life stabilizers, toners, antifoggants, contrast enhancers, development accelerators, acutance dyes, post-processing stabilizers or stabilizer precursors, and other image-modifying agents as would be readily apparent to one skilled in the art.

The photothermographic materials of the present invention can be further protected against the production of fog and can be stabilized against loss of sensitivity during storage. While not necessary for the practice of the invention, it may be advantageous to add mercury (II) salts to the emulsion layer(s) as an antifoggant. Preferred mercury (II) salts for this purpose are mercuric acetate and mercuric bromide. Other useful mercury salts include those described in U.S. Pat. No. 2,728,663 (Allen).

Other suitable antifoggants and stabilizers that can be used alone or in combination include thiazolium salts as described in U.S. Pat. No. 2,131,038 (Staud) and U.S. Pat. No. 2,694,716 (Allen), azaindenes as described in U.S. Pat. No. 2,886,437 (Piper), triazaindolizines as described in U.S. Pat. No. 2,444,605 (Heimbach), the urazoles described in U.S. Pat. No. 3,287,135 (Anderson), sulfocatechols as described in U.S. Pat. No. 3,235,652 (Kennard), the oximes described in GB 623,448 (Carrol et al.), polyvalent metal salts as described in U.S. Pat. No. 2,839,405 (Jones), thiuronium salts as described in U.S. Pat. No. 3,220,839 (Herz), palladium, platinum and gold salts as described in U.S. Pat. No. 2,566,263 (Trirelli) and U.S. Pat. No. 2,597,915 (Damshroder), and 2-(tribromomethylsulfonyl) quinoline compounds as described in U.S. Pat. No. 5,460,938 (Kirk et al.). Stabilizer precursor compounds capable of releasing stabilizers upon application of heat during development can also be used. Such precursor compounds are described in for example, U.S. Pat. No. 5,158,866 (Simpson et al.), U.S. Pat. No. A-5,175,081 (Krepksi et al.), U.S. Pat. No. 5,298,390 (Sakizadeh et al.) and U.S. Pat. No. 5,300,420 (Kenney et al.).

In addition, certain substituted-sulfonyl derivatives of benzotriazoles (for example alkylsulfonylbenzotriazoles and arylsulfonylbenzotriazoles) have been found to be useful stabilizing compounds (such as for post-processing print stabilizing), as described in U.S. Pat. No. 6,171,767 (Kong et al.).

Furthermore, other specific useful antifoggants/stabilizers are described in more detail in U.S. Pat. No. 6,083,681 (Lynch et al.), incorporated herein by reference.

Other antifoggants are hydrobromic acid salts of heterocyclic compounds (such as pyridinium hydrobromide perbromide) as described, for example, in U.S. Pat. No. 5,028,523 (Skoug), compounds having  $-\text{SO}_2\text{CBr}_3$  groups as described for example in U.S. Pat. No. 5,594,143 (Kirk et al.) and U.S. Pat. No. 5,374,514 (Kirk et al.), benzoyl acid compounds as described, for example, in U.S. Pat. No. 4,784,939 (Pham), substituted propenenitrile compounds as described, for example, in U.S. Pat. No. 5,686,228 (Murray et al.), silyl blocked compounds as described, for example,

in U.S. Pat. No. 5,358,843 (Sakizadeh et al.), vinyl sulfones as described, for example, in EP-A-0 600,589 (Philip, Jr. et al.) and EP-A-0 600,586 (Philip, Jr. et al.), and tribromomethylketones as described, for example, in EP-A-0 600,587 (Oliff et al.).

Preferably, the photothermographic materials of this invention include one or more polyhalo antifoggants that include one or more polyhalo substituents including but not limited to, dichloro, dibromo, trichloro, and tribromo groups. The antifoggants can be aliphatic, alicyclic or aromatic compounds, including aromatic heterocyclic and carbocyclic compounds.

The use of "toners" or derivatives thereof that improve the image is highly desirable. Preferably, if used, a toner can be present in an amount of about 0.01% by weight to about 10%, and more preferably about 0.1% by weight to about 10% by weight, based on the total dry weight of the layer in which it is included. Toners may be incorporated in the photothermographic emulsion layer or in an adjacent layer. Toners are well known materials in the photothermographic art, as shown in U.S. Pat. No. 3,080,254 (Grant, Jr.), U.S. Pat. No. 3,847,612 (Winslow), U.S. Pat. No. 4,123,282 (Winslow), U.S. Pat. No. 4,082,901 (Laridon et al.), U.S. Pat. No. 3,074,809 (Owen), U.S. Pat. No. 3,446,648 (Workman), U.S. Pat. No. 3,844,797 (Willems et al.), U.S. Pat. No. 3,951,660 (Hagemann et al.), U.S. Pat. No. 5,599,647 (Defieuw et al.) and GB 1,439,478 (AGFA).

Examples of toners include, but are not limited to, phthalimide and N-hydroxyphthalimide, cyclic imides (such as succinimide), pyrazoline-5-ones, quinazolinone, 1-phenylurazole, 3-phenyl-2-pyrazoline-5-one, and 2,4-thiazolidinedione, naphthalimides (such as N-hydroxy-1,8-naphthalimide), cobalt complexes [such as hexaaminocobalt (3+) trifluoroacetate], mercaptans (such as 3-mercaptop-1,2,4-triazole, 2,4-dimercaptopyrimidine, 3-mercaptop-4,5-diphenyl-1,2,4-triazole and 2,5-dimercapto-1,3,4-thiadiazole), N-(aminomethyl)aryldicarboximides [such as (N,N-dimethylaminomethyl)phthalimide, and N-(dimethylaminomethyl)naphthalene-2,3-dicarboximide, a combination of blocked pyrazoles, isothiuronium derivatives, and certain photobleach agents [such as a combination of N,N'-hexamethylene-bis(1-carbamoyl-3,5-dimethylpyrazole), 1,8-(3,6-diazaoctane)bis(isothiuronium) trifluoroacetate, and 2-(tribromomethylsulfonylbenzothiazole)], merocyanine dyes {such as 3-ethyl-5-[(3-ethyl-2-benzothiazolinylidene)-1-methyl-ethylidene]-2-thio-2,4-o-azolidine-dione}, phthalazine and derivatives thereof [such as those described in U.S. Pat. No. 6,146,822 (Asanuma et al.)], phthalazinone and phthalazinone derivatives, or metal salts or these derivatives [such as 4-(1-naphthyl)phthalazinone, 6-chlorophthalazinone, 5,7-dimethoxyphthalazinone, and 2,3-dihydro-1,4-phthalazinedione], a combination of phthalazine (or derivative thereof) plus one or more phthalic acid derivatives (such as phthalic acid, 4-methylphthalic acid, 4-nitrophthalic acid, and tetrachlorophthalic anhydride), quinazolininediones, benzoxazine or naphthoxazine derivatives, rhodium complexes functioning not only as tone modifiers but also as sources of halide ion for silver halide formation in situ [such as ammonium hexachlororhodate (III), rhodium bromide, rhodium nitrate, and potassium hexachlororhodate (III)], inorganic peroxides and persulfates (such as ammonium peroxydisulfate and hydrogen peroxide), benzoxazine-2,4-diones (such as 1,3-benzoxazine-2,4-dione, 8-methyl-1,3-benzoxazine-2,4-dione and 6-nitro-1,3-benzoxazine-2,4-dione), pyrimidines and asym-triazines (such as 2,4-dihydroxypyrimidine, 2-hydroxy-4-aminopyrimidine and

azauracil) and tetraazapentalene derivatives [such as 3,6-dimercapto-1,4-diphenyl-1H,4H-2,3a,5,6a-tetraazapentalene and 1,4-di-(o-chlorophenyl)-3,6-dimercapto-1H,4H-2,3a,5,6a-tetraazapentalene].

Phthalazines and phthalazine derivatives [such as those described in U.S. Pat. No. 6,146,822 (Asanuma et al.), incorporated herein by reference] are particularly useful toners.

#### Binders

The photocatalyst (such as photosensitive silver halide), the non-photosensitive source of reducible silver ions, the reducing agent composition, and any other additives used in the present invention are generally added to one or more binders that are either hydrophilic or hydrophobic. Thus, either aqueous or solvent-based formulations can be used to prepare the photothermographic materials of this invention. Mixtures of either or both types of binders can also be used. It is preferred that the binder be selected from hydrophobic polymeric materials, such as, for example, natural and synthetic resins that are sufficiently polar to hold the other ingredients in solution or suspension.

Examples of typical hydrophobic binders include, but are not limited to, polyvinyl acetals, polyvinyl chloride, polyvinyl acetate, cellulose acetate, cellulose acetate butyrate, polyolefins, polyesters, polystyrenes, polyacrylonitrile, polycarbonates, methacrylate copolymers, maleic anhydride ester copolymers, butadiene-styrene copolymers, and other materials readily apparent to one skilled in the art. Copolymers (including terpolymers) are also included in the definition of polymers. The polyvinyl acetals (such as polyvinyl butyral and polyvinyl formal) and vinyl copolymers (such as polyvinyl acetate and polyvinyl chloride) are particularly preferred. Particularly suitable binders are polyvinyl butyral resins that are available as BUTVAR® B79 (Solutia, Inc.) and Pioloform BS-18 or Pioloform BL-16 (Wacker Chemical Company).

Examples of useful hydrophilic binders include, but are not limited to, gelatin and gelatin-like derivatives (hardened or unhardened), cellulosic materials such as cellulose acetate, cellulose acetate butyrate, hydroxymethyl cellulose, acrylamide/methacrylamide polymers, acrylic/methacrylic polymers polyvinyl pyrrolidones, polyvinyl acetates, polyvinyl alcohols, and polysaccharides (such as dextrans and starch ethers).

Hardeners for various binders may be present if desired. Useful hardeners are well known and include diisocyanate compounds as described for example in EP-0 600 586B1 and vinyl sulfone compounds as described in EP-0 600 589B1.

Where the proportions and activities of the photothermographic materials require a particular developing time and temperature, the binder(s) should be able to withstand those conditions. Generally, it is preferred that the binder not decompose or lose its structural integrity at 120° C. for 60 seconds. It is more preferred that it not decompose or lose its structural integrity at 177° C. for 60 seconds.

The polymer binder(s) is used in an amount sufficient to carry the components dispersed therein. The effective range can be appropriately determined by one skilled in the art. Preferably, a binder is used at a level of about 10% by weight to about 90% by weight, and more preferably at a level of about 20% by weight to about 70% by weight, based on the total dry weight of the layer in which it is included.

#### Support Materials

The photothermographic materials of this invention comprise a polymeric support that is preferably a flexible, transparent film that has any desired thickness and is com-

posed of one or more polymeric materials, depending upon their use. The supports are generally transparent (especially if the material is used as a photomask) or at least translucent, but in some instances, opaque supports may be useful. They are required to exhibit dimensional stability during thermal development and to have suitable adhesive properties with overlying layers. Useful polymeric materials for making such supports include, but are not limited to, polyesters (such as polyethylene terephthalate and polyethylene naphthalate), cellulose acetate and other cellulose esters, polyvinyl acetal, polyolefins (such as polyethylene and polypropylene), polycarbonates, and polystyrenes (and polymers of styrene derivatives). Preferred supports are composed of polymers having good heat stability, such as polyesters and polycarbonates. Polyethylene terephthalate film is the most preferred support. Various support materials are described, for example, in *Research Disclosure*, August 1979, publication 18431. A method of making dimensionally stable polyester films is described in *Research Disclosure*, September, 1999, publication 42536.

Opaque supports can also be used such as dyed polymeric films and resin-coated papers that are stable to high temperatures.

Support materials can contain various colorants, pigments, antihalation or acutance dyes if desired. Support materials may be treated using conventional procedures (such as corona discharge) to improve adhesion of overlying layers, or subbing or other adhesion-promoting layers can be used. Useful subbing layer formulations include those conventionally used for photographic materials such as vinylidene halide polymers.

#### Photothermographic Formulations

The formulation for the photothermographic emulsion layer(s) can be prepared by dissolving and dispersing the binder, the photocatalyst, the non-photosensitive source of reducible silver ions, the reducing composition, and optional addenda in an organic solvent, such as toluene, 2-butanone, acetone or tetrahydrofuran.

Alternatively, these components can be formulated with a hydrophilic binder in water or water-organic solvent mixtures to provide aqueous-based coating formulations.

Photothermographic materials can contain plasticizers and lubricants such as polyalcohols and diols of the type described in U.S. Pat. No. 2,960,404 (Milton et al.), fatty acids or esters such as those described in U.S. Pat. No. 2,588,765 (Robijns) and U.S. Pat. No. 3,121,060 (Duane), and silicone resins such as those described in GB 955,061 (DuPont). The materials can also contain matting agents such as starch, titanium dioxide, zinc oxide, silica, and polymeric beads including beads of the type described in U.S. Pat. No. 2,992,101 (Jelley et al.) and U.S. Pat. No. 2,701,245 (Lynn). Polymeric fluorinated surfactants may also be useful in one or more layers of the imaging materials for various purposes, such as improving coatability and optical density uniformity as described in U.S. Pat. No. 5,468,603 (Kub).

EP-A-0 792 476 (Geisler et al.) describes various means of modifying the photothermographic materials to reduce what is known as the "woodgrain" effect, or uneven optical density. This effect can be reduced or eliminated by several means, including treatment of the support, adding matting agents to the topcoat, using acutance dyes in certain layers or other procedures described in the noted publication.

The photothermographic materials can include antistatic or conducting layers. Such layers may contain soluble salts (for example chlorides or nitrates), evaporated metal layers, or ionic polymers such as those described in U.S. Pat. No.

2,861,056 (Minsk) and U.S. Pat. No. 3,206,312 (Sterman et al.), or insoluble inorganic salts such as those described in U.S. Pat. No. 3,428,451 (Trevoy), electro-conductive under-layers such as those described in U.S. Pat. No. 5,310,640 (Markin et al.), electronically-conductive metal antimonate particles such as those described in U.S. Pat. No. 5,368,995 (Christian et al.), and electrically-conductive metal-containing particles dispersed in a polymeric binder such as those described in EP-A-0 678 776 (Melpolder et al.). Other antistatic agents are well known in the art.

The photothermographic materials can be constructed of one or more layers on a support. Single layer materials should contain the photocatalyst, the non-photosensitive source of reducible silver ions, the reducing composition, the binder, as well as optional materials such as toners, acutance dyes, coating aids and other adjuvants.

Two-layer constructions comprising a single imaging layer coating containing all the ingredients and a protective topcoat are generally found in the materials of this invention. However, two-layer constructions containing photocatalyst and non-photosensitive source of reducible silver ions in one imaging layer (usually the layer adjacent to the support) and the reducing composition and other ingredients in the second imaging layer or distributed between both layers are also envisioned.

Layers to promote adhesion of one layer to another in photothermographic materials are also known, as described for example in U.S. Pat. No. 5,891,610 (Bauer et al.), U.S. Pat. No. 5,804,365 (Bauer et al.) and U.S. Pat. No. 4,741,992 (Przezdziecki). Adhesion can also be promoted using specific polymeric adhesive materials as described for example in U.S. Pat. No. 5,928,857 (Geisler et al.).

Photothermographic formulations described can be coated by various coating procedures including wire wound rod coating, dip coating, air knife coating, curtain coating, slide coating, or extrusion coating using hoppers of the type described in U.S. Pat. No. 2,681,294 (Beguin). Layers can be coated one at a time, or two or more layers can be coated simultaneously by the procedures described in U.S. Pat. No. 2,761,791 (Russell), U.S. Pat. No. 4,001,024 (Dittman et al.), U.S. Pat. No. 4,569,863 (Keopke et al.), U.S. Pat. No. 5,340,613 (Hanzalik et al.), U.S. Pat. No. 5,405,740 (LaBelle), U.S. Pat. No. 5,415,993 (Hanzalik et al.), U.S. Pat. No. 5,525,376 (Leonard), U.S. Pat. No. 5,733,608 (Kessel et al.), U.S. Pat. No. 5,849,363 (Yapel et al.), U.S. Pat. No. 5,843,530 (Jerry et al.), U.S. Pat. No. 5,861,195 (Bhave et al.) and GB 837,095 (Ilford). A typical coating gap for the emulsion layer can be from about 10 to about 750  $\mu$ m, and the layer can be dried in forced air at a temperature of from about 20° C. to about 100° C. It is preferred that the thickness of the layer be selected to provide maximum image densities greater than about 0.2, and more preferably, from about 0.5 to 5.0 or more, as measured by a MacBeth Color Densitometer Model TD 504.

When the layers are coated simultaneously using various coating techniques, a "carrier" layer formulation comprising a single-phase mixture of the two or more polymers described above may be used. Such formulations are described in copending and commonly assigned U.S. Ser. No. 09/510,648 (filed Feb. 23, 2000 by Ludemann, LaBelle, Geisler, Warren, Crump, and Bhave) that is based on Provisional Application 60/121,794, filed Feb. 26, 1999.

Mottle and other surface anomalies can be reduced in the materials of this invention by incorporation of a fluorinated polymer as described for example in U.S. Pat. No. 5,532,121 (Yonkonski et al.) or by using particular drying techniques as described, for example in U.S. Pat. No. 5,621,983 (Ludemann et al.).

Preferably, two or more layers are applied to a film support using slide coating. The first layer can be coated on top of the second layer while the second layer is still wet. The first and second fluids used to coat these layers can be the same or different organic solvents (or organic solvent mixtures).

While the first and second layers can be coated on one side of the film support, manufacturing methods can also include forming on the opposing or backside of said polymeric support, one or more additional layers, including an antihalation layer, an antistatic layer, or a layer containing a matting agent (such as silica), or a combination of such layers. It is also contemplated that the photothermographic materials of this invention can include emulsion layers on both sides of the support.

To promote image sharpness, photothermographic materials according to the present invention can contain one or more layers containing acutance and/or antihalation dyes. These dyes are chosen to have absorption close to the exposure wavelength and are designed to absorb scattered light. One or more antihalation dyes may be incorporated into one or more antihalation layers according to known techniques, as an antihalation backing layer, as an antihalation underlayer, or as an antihalation overcoat. Additionally, one or more acutance dyes may be incorporated into one or more frontside layers such as the photothermographic emulsion layer, primer layer, underlayer, or topcoat layer according to known techniques. It is preferred that the photothermographic materials of this invention contain an antihalation coating on the support opposite to the side on which the emulsion and topcoat layers are coated.

Dyes particularly useful as antihalation and acutance dyes include dihydroperimidine squaraine dyes having the nucleus represented by the following general Structure X:



Details of such dyes having the dihydroperimidine squaraine nucleus and methods of their preparation can be found in U.S. Pat. No. 6,063,560 (Suzuki et al.) and U.S. Pat. No. 5,380,635 (Gomez et al.), both incorporated herein by reference. These dyes can also be used as acutance dyes in frontside layers of the materials of this invention. One particularly useful dihydroperimidine squaraine dye is cyclobutenediylium, 1,3-bis[2,3-dihydro-2,2-bis[[1-oxohexyl]oxy]methyl]-1H-perimidin-4-yl]-2,4-dihydroxy-, bis(inner salt).

Dyes particularly useful as antihalation dyes in a backside layer of the photothermographic material also include indoline cyanine dyes represented by the following general Structure XI:



XI

Details of such dyes having the indolenine cyanine nucleus and methods of their preparation can be found in EP-A-0 342 810 (Leichter), incorporated herein by reference. One particularly useful cyanine dye, compound (6) described therein, is 3H-Indolium, 2-[2-[2-chloro-3-[(1,3-dihydro-1,3,3-trimethyl-2H-indol-2-ylidene)ethylidene]-5-methyl-1-cyclohexen-1-yl]ethenyl]-1,3,3-trimethyl-, perchlorate.

It is also useful in the present invention to employ acutance or antihalation dyes that will decolorize with heat during processing. Dyes and constructions employing these types of dyes are described in, for example, U.S. Pat. No. 5,135,842 (Kitchin et al.), U.S. Pat. No. 5,266,452 (Kitchin et al.), U.S. Pat. No. 5,314,795 (Helland et al.), and EP-A-0 911 693 (Sakurada et al.).

#### Imaging/Development

While the imaging materials of the present invention can be imaged in any suitable manner consistent with the type of material using any suitable imaging source (typically some type of radiation or electronic signal), the following discussion will be directed to the preferred imaging means. Generally, the materials are sensitive to radiation in the range of from about 300 to about 850 nm.

Imaging can be achieved by exposing the photothermographic materials to a suitable source of radiation to which they are sensitive, including ultraviolet light, visible light, near infrared radiation and infrared radiation to provide a latent image. Suitable exposure means are well known and include laser diodes that emit radiation in the desired region, photodiodes and others described in the art, including *Research Disclosure*, September, 1996, item 38957 (such as sunlight, xenon lamps and fluorescent lamps). Particularly useful exposure means include laser diodes, including laser diodes that are modulated to increase imaging efficiency using what is known as multilongitudinal exposure techniques as described in U.S. Pat. No. 5,780,207 (Mohapatra et al.). Other exposure techniques are described in U.S. Pat. No. 5,493,327 (McCallum et al.).

For using the materials of this invention, development conditions will vary, depending on the construction used but will typically involve heating the imagewise exposed material at a suitably elevated temperature. Thus, the latent image can be developed by heating the exposed material at a moderately elevated temperature of, for example, from about 50 to about 250° C. (preferably from about 80 to about 200° C. and more preferably from about 100 to about 200° C.) for a sufficient period of time, generally from about 1 to about 120 seconds. Heating can be accomplished using any suitable heating means such as a hot plate, a steam iron, a hot roller or a heating bath.

In some methods, the development is carried out in two steps. Thermal development takes place at a higher temperature for a shorter time (for example at about 150° C. for up to 10 seconds), followed by thermal diffusion at a lower temperature (for example at about 80° C.) in the presence of a transfer solvent.

#### Use as a Photomask

The photothermographic materials of the present invention are sufficiently transmissive in the range of from about 350 to about 450 nm in non-imaged areas to allow their use in a process where there is a subsequent exposure of an ultraviolet or short wavelength visible radiation sensitive imageable medium. For example, imaging the photothermographic material and subsequent development affords a visible image. The heat-developed photothermographic material absorbs ultraviolet or short wavelength visible radiation in the areas where there is a visible image and transmits ultraviolet or short wavelength visible radiation where there is no visible image. The heat-developed material may then be used as a mask and positioned between a source of imaging radiation (such as an ultraviolet or short wavelength visible radiation energy source) and an imageable material that is sensitive to such imaging radiation, such as a photopolymer, diazo material, photoresist, or photosensitive printing plate. Exposing the imageable material to the imaging radiation through the visible image in the exposed and heat-developed photothermographic material provides an image in the imageable material. This process is particularly useful where the imageable medium comprises a printing plate and the photothermographic material serves as an imagesetting film.

The following examples are provided to illustrate the practice of this invention, and are not intended to be limiting in any manner. The examples provide exemplary synthetic procedures and preparatory procedures using the combination of chemical sensitizing compounds within the scope of the present invention.

#### Materials and Methods for the Examples:

All materials used in the following examples are readily available from standard commercial sources, such as Aldrich Chemical Co. (Milwaukee Wis.) unless otherwise specified. All percentages are by weight unless otherwise indicated. The following additional terms and materials were used.

ACRYLOID™ A-21 is an acrylic copolymer available from Rohm and Haas (Philadelphia, Pa.).

BUTVAR® B-79 is a polyvinyl butyral resin available from Solutia, Inc. (St. Louis, Mo.).

CAB 171-15S is a cellulose acetate butyrate resin available from Eastman Chemical Co (Kingsport, Tenn.).

DESMODUR® N3300 is an aliphatic hexamethylene diisocyanate available from Bayer Chemicals (Pittsburgh, Pa.).

PERMANAX WSO (or NONOX) is 1,1-bis(2-hydroxy-3,5-dimethylphenyl)-3,5,5-trimethylhexane [CAS RN=7292-14-0] and is available from St-Jean PhotoChemicals, Inc. (Quebec, Canada).

MEK is methyl ethyl ketone (or 2-butanone).

“2-MBO” is 2-mercaptopbenzoxazole (Aldrich Chemical Co.)

“PHP” is pyridinium hydrobromide perbromide.

Sensitizing Dye A is



5

Antifoggant A is 2-(tribromomethylsulfonyl)quinoline and has the following structure:



10

15 Antifoggant B is:



20

25 Backcoat Dye BC-1 is cyclobutenediylium, 1,3-bis[2,3-dihydro-2,2-bis[[1-oxohexyl]oxy]methyl]-1H-perimidin-4-yl]-2,4-dihydroxy-, bis(inner salt). It is believed to have the structure shown below.

BC-1



30

40

Compound HC-1 is described in U.S. Pat. No. 5,545,515 (noted above) and has the following structure:



Vinyl Sulfone-1 (VS-1) is described in U.S. Pat. No. 6,143,487 and has the following structure:

Several comparative gold-containing chemical sensitizers were used in the examples. These compounds are identified in TABLE II below.

TABLE II

| Compound | Au Complex                                                           | Ligand-H (L'-H)  | Method of Preparation or Source                              |
|----------|----------------------------------------------------------------------|------------------|--------------------------------------------------------------|
| C-1      | Au(I)L'Cl                                                            | PPh <sub>3</sub> | Alfa Aesar                                                   |
| C-2      | NaAu(III)Cl <sub>4</sub>                                             |                  | Alfa Aesar                                                   |
| C-3      | [Au(III)L' <sub>2</sub> Br <sub>2</sub> ]<br>[Au(I)Br <sub>2</sub> ] |                  | A. Fabretti et al., J. Chem. Soc., Dalton Trans., 1990, 3091 |
| C-4      | Au(I)L' <sub>2</sub> BF <sub>4</sub>                                 |                  | J. Deaton et al., J. Chem. Soc., Dalton Trans., 1999, 3163   |

TABLE II-continued

| Compound | Au Complex             | Ligand-H (L'-H) | Method of Preparation or Source                               |
|----------|------------------------|-----------------|---------------------------------------------------------------|
| C-5*     | Au(III)L' <sub>3</sub> |                 | M. Gajendragad et al., Bull. Chem. Soc. Japan, 1975, 48, 1024 |

\*This compound is believed to be an Au(I) compound. The elemental analysis and spectral data are consistent with both the Au(III) compound as reported and an Au(I) structure of the type Au(I)L'(HL')<sub>2</sub>. However, the color of the compound is reported to be pale yellow, which is more consistent with an Au(I) compound rather than the usually highly colored yellow-orange Au(III) compounds. Also, a structure of the type Au(I)L'(HL')<sub>2</sub> can be drawn that is chemically and structurally more reasonable than that proposed as an Au(III) compound.

## EXAMPLE 1

The preparation of a photothermographic formulation was carried out as follows:

A preformed silver bromide, silver carboxylate "soap" was prepared as described in U.S. Pat. No. 5,382,504 (noted above), incorporated herein by reference. The average silver halide grain size was 0.12  $\mu\text{m}$ . The photothermographic emulsion was prepared from the soap dispersion in a manner similar to that described in U.S. Pat. No. 6,083,681 (noted above) but using the materials and amounts shown below.

## Photothermographic Emulsion Formulation

To 160 g of this silver soap dispersion at 28.8% solids were added, in order

|                                        |        |
|----------------------------------------|--------|
| ACRYLOID-21 poly(methyl methacrylate)  | 0.58 g |
| CAB 171-15S cellulose acetate butyrate | 14.9 g |
| MEK                                    | 184 g  |
| VS-1                                   | 0.3 g  |
| Benzotriazole                          | 1.6 g  |
| Antifoggant-B                          | 0.12 g |

This green-sensitive imaging formulation was coated under safelight conditions using a dual knife coating machine onto a 7 mil (178  $\mu\text{m}$ ) blue-tinted polyethylene terephthalate support provided with a backside antihalation layer containing Backcoat Dye BC-1 in CAB 171-15S resin binder. Coating and drying were carried out as described in U.S. Pat. No. 6,083,681 (Lynch et al.).

|                                 |                                                                         |
|---------------------------------|-------------------------------------------------------------------------|
| Compound S-VIII-1               | 0.02 g in 5 g of methanol                                               |
| Chemical sensitizer             | 1.2 to 3.16 ml of a 8.9 $\times 10^{-6}$ mol in 50 g of MEK or methanol |
| PHP                             | 0.20 g in 1.58 g of methanol                                            |
| Calcium bromide                 | 0.15 g in 1.19 g of methanol                                            |
| Dye premix formulation          | (see below for ingredients)                                             |
| BUTVAR ® B-79 polyvinyl butyral | 20 g                                                                    |
| Antifoggant A                   | 0.6 g in 10 g of MEK                                                    |
| DESMODUR ® N3300                | 0.63 g in 1.5 g of MEK                                                  |
| Phthalazine                     | 1.0 g in 5 g of MEK                                                     |
| Tetrachlorophthalic acid        | 0.35 g in 2 g of MEK                                                    |
| 4-Methylphthalic acid           | 0.45 g in 4 g of MEK                                                    |
| PERMANAX WSO                    | 10.6 g                                                                  |
| MEK                             | To make 250 g total batch size.                                         |

## Dye Premix Formulation

|                            |        |
|----------------------------|--------|
| Sensitizing Dye A          | 0.02 g |
| Chlorobenzoyl benzoic acid | 1.42 g |
| Methanol                   | 5.0 g  |

## Protective Topcoat Formulation

A protective topcoat for the photothermographic emulsion layer was prepared as follows:

Samples of the resulting green-sensitive photothermographic materials were imagewise exposed for  $10^{-3}$  seconds using an EG&G Flash sensitometer with a P-31 filter and developed using a heated roll processor for 15 seconds at 124° C.

Densitometry measurements were made on a custom built computer-scanned densitometer using a filter appropriate to the sensitivity of the photothermographic material and are believed to be comparable to measurements from commercially available densitometers.  $D_{min}$  is the density of the non-exposed areas after development and it is the average of the eight lowest density values. Speed-1 ("SP-1") is  $\log_1/E+4$  corresponding to the density value of 0.2 above  $D_{min}$  where E is the exposure in ergs/cm<sup>2</sup>. Speed-2 ("SP-2") is  $\log_1/E+4$  corresponding to the density value of 1.00 above  $D_{min}$  where E is the exposure in ergs/cm<sup>2</sup>. Speed-3 ("SP-3") is  $\log_1/E+4$  corresponding to the density value of 2.90 above  $D_{min}$  where E is the exposure in ergs/cm<sup>2</sup>. Average Contrast-1 ("AC-1") is the absolute value of the slope of the line joining the density points at 0.60 and 2.00 above  $D_{min}$ . Contrast-D ("Con-D") is the absolute value of the slope of the line joining the density points at 1.00 and 3.00 above  $D_{min}$ . TABLE III shows the sensitometric data of the resulting photothermographic material. Changes in  $D_{min}$ , SP-1, and SP-2 are relative to a Control photothermographic material having the same composition and structure but from which the gold-containing chemical sensitizer had been omitted.

TABLE III

| Gold-Containing Chemical Sensitizer | Amount (ml) | $\Delta D_{min}$ | $\Delta SP-1$ | $\Delta SP-2$ |
|-------------------------------------|-------------|------------------|---------------|---------------|
| Au-1                                | 3.16        | 0.124            | 0.241         | 0.121         |
| C-1                                 | 3.16        | 0.172            | 0.270         | 0.151         |

5

## EXAMPLE 2

Photothermographic materials like those described in Example 1 were prepared except that they also comprised a surface topcoat over the emulsion layer prepared from the following formulation:

Topcoat Formulation:

|                                        |        |
|----------------------------------------|--------|
| ACRYLOID™ A-21 polymer                 | 0.58 g |
| CAB 171-15S cellulose acetate butyrate | 14.9 g |
| MEK                                    | 184 g  |
| VS-1                                   | 0.3 g  |
| Antifoggant B                          | 0.12 g |
| Benzotriazole                          | 1.6 g  |
| High contrast agent HC-1               | 0.05 g |

10

The green-sensitive photothermographic materials were coated, imaged, and developed as described in Example 1. TABLE IV shows the sensitometric data for the resulting photothermographic material. Changes in  $D_{min}$  and SP-2 are relative to a Control photothermographic material from which the gold chemical sensitizer had been omitted. The materials were found to have a contrast (AC-1) greater than 6.

TABLE IV

| Gold-Containing Chemical Sensitizer | Amount (ml) | $\Delta D_{min}$ | $\Delta SP-1$ | $\Delta SP-2$ |
|-------------------------------------|-------------|------------------|---------------|---------------|
| Au-1                                | 3.16        | 0.092            | 0.400         | 0.376         |
| C-1                                 | 3.16        | 0.152            | 0.542         | 0.494         |

25

## EXAMPLE 3

Green-sensitive photothermographic materials were prepared, imaged, and developed as described in Example 2 except that chemical sensitizer Au-2 was used in the invention material and Compound C-2 was used in the comparative material. Also, the gold-containing chemical sensitizers were added to the imaging formulation after the addition of the calcium bromide. TABLE V shows the sensitometric data for the resulting photothermographic material. Changes in speed and  $D_{min}$  are relative to identically prepared photothermographic materials from which the gold-containing compound had been omitted.

TABLE V

| Gold-Containing Chemical Sensitizer | Amount (ml) | $\Delta D_{min}$ | $\Delta SP-1$ | $\Delta SP-2$ |
|-------------------------------------|-------------|------------------|---------------|---------------|
| Au-2                                | 1.34        | 0.162            | 0.735         | 0.727         |
| C-2                                 | 1.34        | 0.150            | 0.597         | 0.592         |

10

## EXAMPLE 4

Green-sensitive photothermographic materials were prepared, imaged, and developed as described in Example 1 except that Compound C-3 was used in the comparative material. The gold-containing chemical sensitizers were added to the imaging formulation after the addition of the calcium bromide. In addition, the materials were heat developed using a heated roll processor for 12 seconds at 124° C. TABLE VI shows the sensitometric data for the resulting photothermographic material. Changes in speed and  $D_{min}$  are relative to identically prepared photothermographic materials from which the gold-containing compound had been omitted.

25

TABLE VI

| Gold-Containing Chemical Sensitizer | Amount (ml) | $\Delta D_{min}$ | $\Delta SP-1$ | $\Delta SP-2$ |
|-------------------------------------|-------------|------------------|---------------|---------------|
| Au-2                                | 1.26        | 0.149            | 0.392         | 0.235         |
| C-3                                 | 1.26        | 0.110            | 0.134         | 0.071         |

30

35

## EXAMPLE 5

Green-sensitive photothermographic materials were prepared, imaged, and developed as described in Example 2 except that Compound C-3 was used in the comparative material. The gold-containing chemical sensitizers were added to the imaging formulation after the addition of the calcium bromide. TABLE VII shows the sensitometric data for the resulting photothermographic material. Changes in speed and  $D_{min}$  are relative to identically prepared photothermographic materials from which the gold-containing compound had been omitted.

40

45

TABLE VII

| Gold-Containing Chemical Sensitizer | Amount (ml) | $\Delta D_{min}$ | $\Delta SP-1$ | $\Delta SP-2$ |
|-------------------------------------|-------------|------------------|---------------|---------------|
| Au-2                                | 1.26        | 0.153            | 0.671         | 0.670         |
| C-3                                 | 1.26        | 0.148            | 0.305         | 0.310         |

50

55

## EXAMPLE 6

Green-sensitive photothermographic materials were prepared, imaged, and developed as described in Example 2 except that the gold-containing chemical sensitizers were added to the imaging formulation after the addition of the calcium bromide. These materials were found to have a contrast (AC-1) greater than 6. TABLE VIII shows the sensitometric data for the resulting photothermographic material. Changes in speed and  $D_{min}$  are relative to identically prepared photothermographic materials from which

60

65

the gold-containing compound had been omitted.

TABLE VIII

| Gold-Containing Chemical Sensitizer | Amount (ml) | $\Delta D_{min}$ | $\Delta SP-1$ | $\Delta SP-2$ |
|-------------------------------------|-------------|------------------|---------------|---------------|
| Au-1                                | 1.58        | 0.012            | 0.298         | 0.278         |
| C-1                                 | 1.58        | 0.006            | 0.079         | 0.038         |

## EXAMPLE 7

Green-sensitive photothermographic materials were prepared, imaged, and developed as described in Example 1 except that the gold-containing chemical sensitizers were added to the imaging formulation after the addition of the calcium bromide, and iridium- and copper- doped core-shell silver bromide grains (average size of  $0.055\ \mu m$ ) were used. These silver halide grains were prepared as described in U.S. Pat. No. 5,939,249 (noted above). TABLE IX shows the sensitometric data for the resulting photothermographic material. Changes in speed and  $D_{min}$  are relative to identically prepared photothermographic materials from which the gold-containing compound had been omitted.

TABLE IX

| Gold-Containing Chemical Sensitizer | Amount (ml) | $\Delta D_{min}$ | $\Delta SP-1$ | $\Delta SP-2$ |
|-------------------------------------|-------------|------------------|---------------|---------------|
| Au-1                                | 1.70        | 0.017            | 0.189         | 0.108         |
| C-1                                 | 1.70        | 0.018            | 0.029         | -0.008        |
| C-5                                 | 1.58        | -0.011           | 0.004         | -0.047        |

## EXAMPLE 8

Green-sensitive photothermographic materials were prepared, imaged, and developed as described in Example 7 except that the materials also had a topcoat layer prepared as described in Example 2. The materials were found to have a contrast (AC-1) greater than 6. TABLE X shows the sensitometric data for the resulting photothermographic material. Changes in speed and  $D_{min}$  are relative to identically prepared photothermographic materials from which the gold-containing compound had been omitted. The data also show that the use of chemical sensitizer C-5 provided essentially no speed increase in the photothermographic materials.

TABLE X

| Gold-Containing Chemical Sensitizer | Amount (ml) | $\Delta D_{min}$ | $\Delta SP-1$ | $\Delta SP-2$ |
|-------------------------------------|-------------|------------------|---------------|---------------|
| Au-1                                | 1.70        | 0.008            | 0.266         | 0.248         |
| C-1                                 | 1.70        | 0.013            | 0.111         | 0.105         |
| C-5                                 | 1.58        | -0.007           | 0.030         | 0.024         |

## EXAMPLE 9

Green-sensitive photothermographic materials were prepared, imaged, and developed as described in Example 1 except gold(III)-containing Compound Au-2 was used and the gold-containing chemical sensitizers were added to the

imaging formulation after the addition of the calcium bromide. TABLE XI shows the sensitometric data for the resulting photothermographic material. Changes in speed and  $D_{min}$  are relative to identically prepared photothermographic materials from which the gold-containing compound had been omitted. The data show that the material of the present invention provided a higher ratio of the change in speed to the change in  $D_{min}$  compared to the material containing compounds C-2 or C-4. The data also show that the use of chemical sensitizer compound C-5 in higher amounts provided essentially no speed increase.

TABLE XI

| Gold-Containing Chemical Sensitizer | Amount (ml) | $\Delta D_{min}$ | $\Delta SP-1$ | $\Delta SP-2$ |
|-------------------------------------|-------------|------------------|---------------|---------------|
| Au-2                                | 1.50        | 0.181            | 0.490         | 0.455         |
| C-2                                 | 1.50        | 0.190            | 0.346         | 0.326         |
| C-4                                 | 1.50        | 0.442            | 0.590         | 0.509         |
| C-4                                 | 1.26        | 0.317            | 0.389         | 0.378         |
| C-5                                 | 3.16        | 0.36             | 0.160         | -0.015        |

## EXAMPLE 10

Green-sensitive photothermographic materials were prepared, imaged, and developed as described in Example 2 except gold(III)-containing Compound Au-2 was used and the gold-containing chemical sensitizers were added to the imaging formulation after the addition of the calcium bromide. TABLE XII shows the sensitometric data for the resulting photothermographic material. Changes in speed and  $D_{min}$  are relative to identically prepared photothermographic materials from which the gold-containing compound had been omitted.

TABLE XII

| Gold-Containing Chemical Sensitizer | Amount (ml) | $\Delta D_{min}$ | $\Delta SP-1$ | $\Delta SP-2$ |
|-------------------------------------|-------------|------------------|---------------|---------------|
| Au-2                                | 1.50        | 0.175            | 0.858         | 0.815         |
| C-2                                 | 1.50        | 0.184            | 0.761         | 0.711         |
| C-4                                 | 1.50        | fogged           | —             | —             |
| C-4                                 | 1.26        | fogged           | —             | —             |
| C-5                                 | 3.16        | fogged           | —             | —             |

## EXAMPLE 11

50 A photothermographic formulation was prepared as follows: A 93% silver carboxylate “soap” was dispersed in MEK. The “soap” contained a mixture of C-18, C-20 and C-22 chain length silver carboxylates. To 550 g of this silver soap dispersion was added 37.5 g of BUTVAR® B-79 poly(vinyl butyral) resin and 191.3 g of MEK, followed by homogenization to 23.5% solids.

The silver halide emulsion was prepared by precipitation by mixing lithium bromide, silver trifluoroacetate, and poly (vinyl butyral) in acetone under controlled conditions to 55 yield silver bromide grains having an average size of  $0.079\ \mu m$ . This procedure is known in the art as an ex-situ silver halide preparation and has been described, for example, in U.S. Pat. No. 3,871,887 (incorporated herein by reference). To 9 g of this emulsion were added compound S-IV-50 (1.59 ml of a  $2.5 \times 10^{-5}$  mole solution in 25 g of methanol) and the gold-containing chemical sensitizer (0.79 ml of a  $8.7 \times 10^{-6}$  mole solution in 25 g of methanol).

## Photothermographic Emulsion Formulation:

To 190 g of the noted silver soap dispersion at 23.5% solids were added, in order:

|                                    |                                                |
|------------------------------------|------------------------------------------------|
| PHP                                | 0.20 g in 1.58 g of methanol                   |
| Calcium bromide                    | 0.15 g in 1.19 g of methanol                   |
| Silver halide emulsion noted above | 9 g (21.7% solids) (see below for ingredients) |
| Dye premix                         | 20 g                                           |
| BUTVAR ® B-79 poly(vinyl butyral)  | 0.6 g in 10 g of MEK                           |
| Antifogant A                       | 0.63 g in 1.5 g of MEK                         |
| DESMODUR ® N3300                   | 1.0 g in 5 g of MEK                            |
| Phthalazine                        | 0.35 g in 2 g of MEK                           |
| Tetrachlorophthalic acid           | 0.45 g in 4 g of MEK                           |
| 4-Methylphthalic acid              | 10.6 g                                         |
| PERMANAX WSO                       | To make 250 g total batch size.                |
| MEK                                |                                                |
| Dye Premix Formulation:            |                                                |
| Sensitizing Dye A                  | 0.02 g                                         |
| Chlorobenzoyl benzoic acid         | 1.42 g                                         |
| Methanol                           | 5.0 g                                          |

A topcoat formulation was prepared as described in Example 2. The resulting green-sensitive photothermographic materials were prepared, imaged, and heat-developed as described in Example 1. They were shown to have a contrast (AC-1) greater than 6. TABLE XIII shows the sensitometric data for the resulting photothermographic material. Changes in speed and  $D_{min}$  are relative to identically prepared photothermographic materials from which the gold-containing compound had been omitted.

TABLE XIII

| Gold-Containing Chemical Sensitizer | Amount (ml) | $\Delta D_{min}$ | $\Delta SP-1$ | $\Delta SP-2$ |
|-------------------------------------|-------------|------------------|---------------|---------------|
| Au-1                                | 0.79        | 0.030            | 0.165         | 0.137         |
| C-1                                 | 0.79        | 0.031            | 0.060         | 0.037         |

Similar photothermographic materials were prepared as described in this example except that either no chemical sensitizers were included or only Compound Au-1 or C-1 was included (that is, no additional sulfur- or tellurium-containing compound was present). In addition, for the first two comparative materials (noted with \*), the topcoat did not include the high contrast agent HC-1. TABLE XIV shows the sensitometric data for the resulting photothermographic material. Changes in speed and  $D_{min}$  are relative to identically prepared photothermographic materials from which the gold-containing compound had been omitted. No speed increase was observed with either material containing only the gold chemical sensitizer.

TABLE XIV

| Gold-Containing Chemical Sensitizer | Amount (ml) | $\Delta D_{min}$ | $\Delta SP-1$ | $\Delta SP-2$ |
|-------------------------------------|-------------|------------------|---------------|---------------|
| Au-1*                               | 0.79        | -0.008           | -0.060        | -0.017        |
| C-1*                                | 0.79        | -0.008           | -0.025        | 0.007         |

TABLE XIV-continued

| Gold-Containing Chemical Sensitizer | Amount (ml) | $\Delta D_{min}$ | $\Delta SP-1$ | $\Delta SP-2$ |
|-------------------------------------|-------------|------------------|---------------|---------------|
| Au-1                                | 0.79        | -0.005           | -0.116        | -0.116        |
| C-1                                 | 0.79        | -0.002           | -0.049        | -0.049        |

## EXAMPLE 12

A green-sensitive photothermographic material was prepared, imaged, and heat-developed as described in Example 11 except that the gold-containing chemical sensitizer was provided in 0.167 g of the following solution:

## Chemical Sensitizer Solution:

|                                   |                                  |
|-----------------------------------|----------------------------------|
| Chemical sensitizer               | 0.0188 g in 7.5 g of water       |
| BUTVAR ® B-76 poly(vinyl butyral) | 18.5 g of 5% solution in toluene |
| Benzyl alcohol                    | 1.15 g                           |

The topcoat was prepared without high contrast agent HC-1. TABLE XV shows the resulting sensitometric data for this material. The changes in speed and  $D_{min}$  are relative to an identically prepared photothermographic material prepared from which the gold-containing compound had been omitted.

TABLE XV

| Gold-Containing Chemical Sensitizer | Amount (g) | $\Delta D_{min}$ | $\Delta SP-1$ | $\Delta SP-2$ |
|-------------------------------------|------------|------------------|---------------|---------------|
| Au-2                                | 0.0167     | 0.113            | 0.559         | 0.470         |

## EXAMPLE 13

A green-sensitive photothermographic material was prepared, imaged, and heat-developed as described in Example 12 except that the topcoat was prepared as described in Example 11. The material was found to have a contrast (AC-1) greater than 6. TABLE XVI shows the sensitometric data for the resulting photothermographic material. Changes in speed and  $D_{min}$  are relative to identically prepared photothermographic materials from which the gold-containing compound had been omitted. The change in speed relative to the change in  $D_{min}$  was high.

TABLE XVI

| Gold-Containing Chemical Sensitizer | Amount (g) | $\Delta D_{min}$ | $\Delta SP-1$ | $\Delta SP-2$ |
|-------------------------------------|------------|------------------|---------------|---------------|
| Au-2                                | 0.0167     | 0.118            | 0.702         | 0.667         |

## EXAMPLE 14

Green-sensitive photothermographic materials were prepared, imaged, and heat-developed as described in Example 1 except that the gold-containing chemical sensi-

tizers were added to the imaging formulation after the addition of the calcium bromide. TABLE XVII shows the sensitometric data for the resulting photothermographic material. Changes in speed and  $D_{min}$  are relative to identically prepared photothermographic materials from which the gold-containing chemical sensitizer had been omitted.

TABLE XVII

| Gold-Containing Chemical Sensitizer | Amount (ml) | $\Delta D_{min}$ | ASP-1 | ASP-2 |
|-------------------------------------|-------------|------------------|-------|-------|
| Au-2                                | 1.58        | 0.095            | 0.352 | 0.293 |
| Au-3                                | 1.58        | 0.113            | 0.297 | 0.214 |
| Au-4                                | 1.42        | 0.259            | 0.411 | 0.299 |
| Au-5                                | 1.34        | 0.217            | 0.356 | 0.287 |

## EXAMPLE 15

Green-sensitive photothermographic materials were prepared, imaged, and developed as described in Example 2 except that the gold-containing chemical sensitizers were added to the imaging formulation after the addition of the calcium bromide. The materials were found to have a contrast (AC-1) greater than 6. TABLE XVIII shows the sensitometric data for the resulting photothermographic material. Changes in speed and  $D_{min}$  are relative to identically prepared photothermographic materials from which the gold-containing compound had been omitted.

TABLE XVIII

| Gold-Containing Chemical Sensitizer | Amount (ml) | $\Delta D_{min}$ | ASP-1 | ASP-2 |
|-------------------------------------|-------------|------------------|-------|-------|
| Au-2                                | 1.58        | 0.080            | 0.494 | 0.472 |
| Au-3                                | 1.58        | 0.111            | 0.455 | 0.433 |
| Au-4                                | 1.42        | 0.196            | 0.672 | 0.627 |
| Au-5                                | 1.34        | 0.156            | 0.560 | 0.538 |

## EXAMPLE 16

Green-sensitive photothermographic materials were prepared, imaged, and developed as described in Example 6 except that the topcoat did not contain the high contrast agent HC-1. TABLE XIX shows the sensitometric data for the resulting photothermographic material. Changes in speed and  $D_{min}$  are relative to identically prepared photothermographic materials from which the gold-containing compound had been omitted.

TABLE XIX

| Gold-Containing Chemical Sensitizer | Amount (ml) | $\Delta D_{min}$ | ASP-1 | ASP-2 |
|-------------------------------------|-------------|------------------|-------|-------|
| Au-2                                | 1.58        | 0.071            | 0.476 | 0.334 |
| Au-4                                | 1.58        | 0.064            | 0.439 | 0.290 |
| Au-6                                | 1.58        | 0.040            | 0.385 | 0.219 |

## EXAMPLE 17

Green-sensitive photothermographic materials were prepared, imaged, and developed as described in Example 6. They were found to have a contrast (AC-1) greater than 6.

TABLE XX shows the sensitometric data for the resulting photothermographic material. Changes in speed and  $D_{min}$  are relative to identically prepared photothermographic materials from which the gold-containing compound had been omitted.

TABLE XX

| Gold-Containing Chemical Sensitizer | Amount (ml) | $\Delta D_{min}$ | ASP-1 | ASP-2 |
|-------------------------------------|-------------|------------------|-------|-------|
| Au-2                                | 1.58        | 0.058            | 0.663 | 0.603 |
| Au-4                                | 1.58        | 0.047            | 0.554 | 0.517 |
| Au-6                                | 1.58        | 0.028            | 0.422 | 0.390 |

## EXAMPLE 18

A green-sensitive photothermographic material was prepared, imaged, and developed as described in Example 7. TABLE XXI shows the sensitometric data for the resulting photothermographic material. Changes in speed and  $D_{min}$  are relative to an identically prepared photothermographic material from which the gold-containing compound had been omitted.

TABLE XXI

| Gold-Containing Chemical Sensitizer | Amount (ml) | $\Delta D_{min}$ | ASP-1 | ASP-2 |
|-------------------------------------|-------------|------------------|-------|-------|
| Au-2                                | 1.43        | 0.063            | 0.368 | 0.249 |

## EXAMPLE 19

A green-sensitive photothermographic material was prepared, imaged, and developed as described in Example 8. It was shown to have a contrast (AC-1) greater than 6. TABLE XXII shows the sensitometric data for the resulting photothermographic material. Changes in speed and  $D_{min}$  are relative to an identically prepared photothermographic material from which the gold-containing compound had been omitted.

TABLE XXII

| Gold-Containing Chemical Sensitizer | Amount (ml) | $\Delta D_{min}$ | ASP-1 | ASP-2 |
|-------------------------------------|-------------|------------------|-------|-------|
| Au-2                                | 1.43        | 0.054            | 0.517 | 0.491 |

## EXAMPLE 20

This example demonstrates the effect of a combination of tellurium-containing and gold(III)-containing chemical sensitizers in photothermographic materials using iridium-doped core-shell silver halide grains prepared as described in U.S. Pat. No. 5,434,043 (noted above). The silver halide grains were sensitized using a red sensitizing dye and high contrast agent HC-1. All of the materials provided a "Con-D" greater than 10.

## Photothermographic Emulsion Formulation:

To 176 g of the silver soap dispersion at 28.2% solids containing 46 g of preformed "soap" were added, in order:

|                                     |                                                                                   |
|-------------------------------------|-----------------------------------------------------------------------------------|
| MEK                                 | 14 g                                                                              |
| PHP                                 | 0.2544 g                                                                          |
| Zinc bromide                        | 0.288 g                                                                           |
| Tellurium Compound Te-II-1          | 0.0139 g                                                                          |
| Gold (III) chemical sensitizer Au-2 | 3 g of $8.5 \times 10^{-6}$ mole in 250 g of methanol (see below for ingredients) |
| Dye premix formulation              | 31.8 g                                                                            |
| BUTVAR ® B-79 poly(vinyl butyral)   | 1.6 g                                                                             |
| Antifoggant A                       | 0.49 g                                                                            |
| DESMODUR ® N3300                    | 1.2 g                                                                             |
| Phthalazine                         | 0.27 g                                                                            |
| Tetrachlorophthalic acid            | 0.60 g                                                                            |
| 4-Methylphthalic acid               | 12.0 g                                                                            |
| PERMANAX WSO                        | 0.215 g                                                                           |
| High contrast agent HC-1            |                                                                                   |

## Dye Premix Formulation:

|                            |              |
|----------------------------|--------------|
| Sensitizing dye C          | 0.02368 mmol |
| Chlorobenzoyl benzoic acid | 2.32 g       |
| 2-Mercaptobenzoxazole      | 0.014 g      |
| Methanol                   | 9.82 g       |

  

|                                        |         |
|----------------------------------------|---------|
| ACRYLOID™ A-21 polymer                 | 0.052 g |
| CAB 171-15S cellulose acetate butyrate | 1.34 g  |
| MEK                                    | 16.95 g |
| VS-1                                   | 0.079 g |

## Topcoat Formulation:

A topcoat formulation (20 g) was prepared as follows:

5 mide grains were used as seed grains to grow grains to a final average size of 0.12  $\mu\text{m}$  using the procedure described in U.S. Pat. No. 3,871,887. To 12.8 g of this emulsion were added 0.79 ml of a solution containing  $2.72 \times 10^{-5}$  mole of sulfur-containing chemical sensitizer S-IV-50 in 25 g of methanol and 0.26 ml of a solution containing  $8.5 \times 10^{-6}$  mole of gold-containing chemical sensitizer Au-2 in 25 g of methanol. After the addition of these chemical sensitizers a dye premix formulation containing 0.02 g of sensitizing Dye A in 5.0 g of methanol was added.

## Photothermographic Emulsion Formulation:

10 To 199 g of this silver soap dispersion at 23.5% solids was added:

|                                    |                                 |
|------------------------------------|---------------------------------|
| PHP                                | 0.20 g in 1.58 g of methanol    |
| Calcium bromide                    | 0.15 g in 1.19 g of methanol    |
| Chlorobenzoyl benzoic acid         | 1.42 g                          |
| BUTVAR ® B-79 poly(vinyl butyral)  | 20 g                            |
| Antifoggant-A                      | 0.6 g in 10 g of MEK            |
| DESMODUR ® N3300                   | 0.63 g in 1.5 g of MEK          |
| Phthalazine                        | 1.00 g in 5.0 g of MEK          |
| Tetrachlorophthalic acid           | 0.35 g in 2.0 g of MEK          |
| 4-methylphthalic acid              | 0.45 g in 4.0 g of MEK          |
| PERMANAX WSO                       | 10.6 g                          |
| Silver halide emulsion noted above | 12.8 g                          |
| MEK                                | To make 250 g total batch size. |

35 The photothermographic material of this invention was prepared by coating these formulations under safelight conditions onto a 4 mil (102  $\mu\text{m}$ ) polyethylene terephthalate support provided with a backside antihalation layer containing a dye having an absorbance >1.0 at the imaging wavelength of exposure (670 nm). Coating and drying were carried out using a dual-knife coating machine and as described in U.S. Pat. No. 6,083,681 (Lynch et al.).

40 Samples of the resulting red-sensitive photothermographic materials were imagewise exposed using a conventional laser scanning sensitometer comprising a 670 nm laser diode. The materials were then heat-developed using a heated roll processor for 13 seconds at 118° C.

45 Sensitometric results were obtained as described in the previous examples in comparison to a material from which the gold(III)-containing chemical had been omitted. The results are shown in TABLE XXII below. The material of this invention provided the desired speed increase with little increase in  $D_{min}$ .

TABLE XXIII

| Gold-Containing Chemical Sensitizer | Amount (g) | $\Delta D_{min}$ | $\Delta SP-3$ |
|-------------------------------------|------------|------------------|---------------|
| Au-2                                | 3.00       | 0.041            | 0.243         |

## EXAMPLE 21

Photothermographic materials were prepared like those described in Example 11 except that 0.079  $\mu\text{m}$  silver bro-

5 mide grains were used as seed grains to grow grains to a final average size of 0.12  $\mu\text{m}$  using the procedure described in U.S. Pat. No. 3,871,887. To 12.8 g of this emulsion were added 0.79 ml of a solution containing  $2.72 \times 10^{-5}$  mole of sulfur-containing chemical sensitizer S-IV-50 in 25 g of methanol and 0.26 ml of a solution containing  $8.5 \times 10^{-6}$  mole of gold-containing chemical sensitizer Au-2 in 25 g of methanol. After the addition of these chemical sensitizers a dye premix formulation containing 0.02 g of sensitizing Dye A in 5.0 g of methanol was added.

## Photothermographic Emulsion Formulation:

10 To 199 g of this silver soap dispersion at 23.5% solids was added:

|                                    |                                 |
|------------------------------------|---------------------------------|
| PHP                                | 0.20 g in 1.58 g of methanol    |
| Calcium bromide                    | 0.15 g in 1.19 g of methanol    |
| Chlorobenzoyl benzoic acid         | 1.42 g                          |
| BUTVAR ® B-79 poly(vinyl butyral)  | 20 g                            |
| Antifoggant-A                      | 0.6 g in 10 g of MEK            |
| DESMODUR ® N3300                   | 0.63 g in 1.5 g of MEK          |
| Phthalazine                        | 1.00 g in 5.0 g of MEK          |
| Tetrachlorophthalic acid           | 0.35 g in 2.0 g of MEK          |
| 4-methylphthalic acid              | 0.45 g in 4.0 g of MEK          |
| PERMANAX WSO                       | 10.6 g                          |
| Silver halide emulsion noted above | 12.8 g                          |
| MEK                                | To make 250 g total batch size. |

35 A topcoat formulation was prepared and coated as described in Example 2.

40 The resulting green-sensitive photothermographic materials were prepared, imaged, and heat-developed as described in Example 1. They were found to have an average contrast (AC-1) greater than 4. TABLE XXV shows the sensitometric data for this photothermographic material. The changes in speed and  $D_{min}$  are relative to an identically prepared photothermographic material from which the gold-containing compound had been omitted.

TABLE XXIV

| Gold-Containing Chemical Sensitizer | Amount (ml) | $\Delta D_{min}$ | $\Delta SP-1$ | $\Delta Speed-2$ |
|-------------------------------------|-------------|------------------|---------------|------------------|
| Au-2                                | 0.26        | -0.044           | 0.360         | 0.465            |

## EXAMPLE 22

60 Green-sensitive photothermographic materials were prepared, imaged and developed as described in Example 8 except that 1.26 ml of a solution containing of  $4.41 \times 10^{-5}$  moles of sulfur-containing chemical sensitizer S-IV-2 in 5.0 g of methanol was added to the imaging formulation after the addition of calcium bromide and gold-containing chemical sensitizer Au-2 was used. The samples were developed for 10 seconds at 124° C.

The materials were found to have an average contrast (AC-1) greater than 6. TABLE XXV shows the sensitometric data for this photothermographic material. The changes in speed and  $D_{min}$  are relative to an identically prepared photothermographic material from which the gold-containing compound had been omitted.

TABLE XXV

| Gold-Containing Chemical Sensitizer | Amount (ml) | $\Delta D_{min}$ | $\Delta SP-1$ | $\Delta Speed-3$ |
|-------------------------------------|-------------|------------------|---------------|------------------|
| Au-2                                | 1.26        | 0.041            | 0.428         | 0.386            |

The invention has been described in detail with particular reference to certain preferred embodiments thereof, but it will be understood that variations and modifications can be effected within the spirit and scope of the invention.

We claim:

1. A photothermographic material comprising a support having thereon one or more layers comprising a hydrophobic binder and in reactive association:

- photosensitive silver halide grains,
- a non-photosensitive source of reducible silver ions, and
- a reducing composition for said reducible silver ions, wherein said photosensitive silver halide grains have been chemically sensitized with a combination of chemical sensitizers that consists essentially of a sulfur- or tellurium-containing compound, and a gold(III)-containing compound that is represented by the following Structure GOLD:



## GOLD

wherein  $L'$  represents the same or different ligands, each ligand comprising at least one heteroatom that is capable of forming a bond with gold,  $Y$  is an anion,  $r$  is an integer of from 1 to 8, and  $q$  is an integer of from 0 to 3.

2. The photothermographic material of claim 1 wherein the molar ratio of said sulfur- or tellurium-containing compound to said gold(III)-containing compound is from about 10,000:1 to 1:10.

3. The photothermographic material of claim 1 wherein said silver halide is chemically sensitized with said sulfur- or tellurium-containing compound in an amount of from about  $10^{-8}$  to about  $10^{-2}$  mole per mole of total silver and with said gold(III)-containing compound in an amount of from about  $10^{-10}$  to about  $10^{-2}$  mole per mole of total silver.

4. The photothermographic material of claim 1 wherein  $L'$  represents the same or different ligands that comprise at least one oxygen, nitrogen, sulfur, or phosphorous atom.

5. The photothermographic material of claim 4 wherein  $L'$  is pyridine, bipyridine, terpyridine,  $P(phenyl)_3$ , carboxylate, imine, phenol, mercaptophenol, imidazole, triazole, and dithioxamide.

6. The photothermographic material of claim 1 wherein  $Y$  is a halide,  $r$  is an integer of from 1 to 3, and  $q$  is 3.

7. The photothermographic material of claim 1 wherein said gold(III)-containing compound is one or more of Compounds Au-1 to Au-14.

| Compound | Au(III) Complex      | Ligand-H ( $L'-H$ )                                                                   |
|----------|----------------------|---------------------------------------------------------------------------------------|
| Au-1     | $AuL'ClBr_2$         | $P(phenyl)_3$                                                                         |
| Au-2     | $AuL'Cl_3$           |    |
| Au-3     | $AuL'Br_2$           |    |
| Au-4     | $AuL'Cl_3$           |    |
| Au-5     | $L[AuP(phenyl)_3]_3$ |    |
| Au-6     | $AuL'Cl_3$           |  |
| Au-7     | $AuH(L')_2Cl_2$      |  |
| Au-8     | $AuL'Cl_2$           |  |
| Au-9     | $Au_2Zn(L')_8$       |  |
| Au-10    | $AuPF_6(L')_2$       |  |
| Au-11    | $Au(L')_2Br$         |  |

-continued

| Compound | Au(III) Complex                          | Ligand-H (L'-H)                                                                   |
|----------|------------------------------------------|-----------------------------------------------------------------------------------|
| Au-12    | $\text{AuL}'\text{Cl}_3$                 |  |
| Au-13    | $\text{Au}(\text{L}')_2(\text{ClO}_4)_3$ |                                                                                   |
| Au-14    | $\text{AuL}'\text{Cl}$                   | Diferrocenylphenylphosphine<br>Glycylglycyl-L-histidine                           |

8. The photothermographic material of claim 1 wherein the tellurium-containing compound is represented by the following Structure I, II or III:



wherein X represents a COR, CSR, CN(R)<sub>2</sub>, CR, P(R)<sub>2</sub>, or P(OR)<sub>2</sub> group, R is an alkyl, alkenyl, or aryl group, L represents the same or different ligand derived from a neutral Lewis base, X<sup>1</sup> and X<sup>2</sup> represent a halo, OCN, SCN, S<sub>2</sub>CN(R)<sub>2</sub>, S<sub>2</sub>COR, S<sub>2</sub>CSR, S<sub>2</sub>P(OR)<sub>2</sub>, S<sub>2</sub>P(R)<sub>2</sub>, SeCN, TeCN, CN, SR, OR, N<sub>3</sub>, alkyl, aryl, or O<sub>2</sub>CR group, R' is an alkyl or aryl group, p is 2 or 4, m is 0, 1, 2, or 4, and n is 2 or 4, provided that when m is 0 or 2, n is 2 or 4, and when m is 1 or 4, n is 2.

9. The photothermographic material of claim 8 wherein L represents the same or different ligands derived from thiourea, a substituted thiourea, pyridine, or a substituted pyridine group.

10. The photothermographic material of claim 1 that further comprises a merocyanine spectral sensitizing dye and said photosensitive silver halide is chemically sensitized with a tellurium-containing compound in combination with said gold(III)-containing compound.

11. The photothermographic material of claim 1 wherein said photosensitive silver halide is chemically sensitized with a sulfur-containing compound that is represented by the following Structure IV, V, or VI:



-continued



wherein:

in Structure IV, R<sub>1</sub>, R<sub>2</sub>, R<sub>3</sub> and R<sub>4</sub> are independently hydrogen, alkyl, cycloalkyl, allyl, alkenyl, alkynyl, aryl or heterocyclic groups, or R<sub>1</sub> and R<sub>2</sub> taken together, R<sub>3</sub> and R<sub>5</sub> taken together, R<sub>1</sub> and R<sub>3</sub> taken together or R<sub>2</sub> and R<sub>4</sub> taken together, can form a 5- to 7-membered heterocyclic ring,

in Structure V, R<sub>1</sub>, R<sub>2</sub>, R<sub>3</sub>, R<sub>4</sub> and R<sub>5</sub> are independently hydrogen, alkyl, cycloalkyl, allyl, alkenyl, alkynyl, aryl or heterocyclic groups, or R<sub>3</sub> and R<sub>5</sub> taken together, R<sub>4</sub> and R<sub>5</sub> taken together, R<sub>1</sub> and R<sub>3</sub> taken together or R<sub>2</sub> and R<sub>4</sub> taken together, can form a substituted or unsubstituted 5- to 7-membered heterocyclic ring, and

in Structure VI, R<sub>1</sub>, R<sub>2</sub>, R<sub>3</sub>, R<sub>4</sub>, R<sub>5</sub>, and R<sub>6</sub> are independently hydrogen, alkyl, cycloalkyl, allyl, alkenyl, alkynyl, aryl or heterocyclic groups, or R<sub>3</sub> and R<sub>6</sub> taken together, R<sub>4</sub> and R<sub>5</sub> taken together, R<sub>1</sub> and R<sub>3</sub> taken together, R<sub>2</sub> and R<sub>4</sub> taken together, or R<sub>5</sub> and R<sub>6</sub> taken together, can form a substituted or unsubstituted 5- to 7-membered heterocyclic ring, and R<sub>7</sub> is a divalent aliphatic or alicyclic linking group.

12. The photothermographic material of claim 11 wherein said photosensitive silver halide is chemically sensitized with a sulfur-containing compound that is a 1,1,3,3-tetr subsituted thiourea having an acid group with an acid dissociation constant (pKa) of less than 7.

13. The photothermographic material of claim 1 wherein said photosensitive silver halide has been chemically sensitized by decomposition of a sulfur-containing compound on or around the grains thereof in an oxidizing environment.

14. The photothermographic material of claim 1 wherein said photosensitive silver halide is chemically sensitized with a sulfur-containing compound containing a thiohydantoin, rhodanine, or 2-thio-4-oxo-oxazolidine nucleus that is represented by the following Structure VII, VIII, or IX:



15. The photothermographic material of claim 1 wherein said non-photosensitive source of reducible silver ions is a

silver salt of a fatty acid having from 10 to 30 carbon atoms, or a mixture of said silver salts.

16. The photothermographic material of claim 1 further comprising a co-developer.

17. The photothermographic material of claim 16 wherein said co-developer is selected from the group consisting of trityl hydrazides, formyl phenyl hydrazides, 3-heteroaromatic-substituted acrylonitriles, 2-substituted malondialdehyde compounds, substituted propenitriles, 4-substituted isoxazoles, 2,5-dioxo-cyclopentane carboxaldehydes, 5-(hydroxymethylene)-1,3-dialkylbarbituric acids, and 2-(ethoxymethylene)-1H-indene-1,3(2H)-diones. 10

18. The photothermographic material of claim 17 further including a contrast enhancing agent.

19. The photothermographic material of claim 18 wherein said contrast enhancing agent is selected from the group consisting of hydroxylamines, alkanolamines, ammonium phthalamate compounds, hydroxamic acid compounds, N-acylhydrazine compounds, and hydrogen atom donor compounds. 15

20. The photothermographic material of claim 1 further comprising a heteroaromatic mercapto compound in an amount of at least 0.0001 mole per mole of total silver. 25

21. The photothermographic material of claim 20 wherein said heteroaromatic mercapto compound is 2-mercaptopbenzimidazole, 2-mercaptop-5-methylbenzimidazole, 2-mercaptopbenzothiazole, 2-mercaptopbenzoxazole, or a mixture of two or more of these compounds. 30

22. The photothermographic material of claim 1 wherein said photosensitive silver halide is chemically sensitized with a mixture of gold-containing compounds, at least 25 mol % of which are gold(III)-containing compounds represented by Structure GOLD. 35

23. The photothermographic material of claim 1 further comprising a dihydroperimidine squaraine dye having a nucleus represented by the following Structure X: 40



24. The photothermographic material of claim 1 wherein said dihydroperimidine squaraine dye is cyclobutenediylium, 1,3-bis[2,3-dihydro-2,2-bis[[1-oxohexyl]oxy]methyl]-1H-perimidin-4-yl]-2,4-dihydroxy-, bis(inner salt) that is present as an antihalation or acutance dye. 60

25. The photothermographic material of claim 1 further comprising a backside antihalation layer comprising an indolene cyanine antihalation dye having a nucleus represented by the following Structure XI: 65



26. A method for forming a visible image comprising:

A) imagewise exposing the photothermographic material of claim 1 to electromagnetic radiation to form a latent image, and

B) simultaneously or sequentially, heating said exposed photothermographic material to develop said latent image into a visible image.

27. The method of claim 26 wherein said photothermographic material support is transparent, and said method further comprises:

C) positioning said exposed and heat-developed photothermographic material with a visible image therein between a source of imaging radiation and an imageable material that is sensitive to said imaging radiation, and

D) thereafter exposing said imageable material to said imaging radiation through said visible image in said exposed and heat-developed photothermographic material to provide a visible image in said imageable material.

28. A method of preparing a photothermographic emulsion comprising:

A) providing a photothermographic emulsion comprising photosensitive silver halide grains and a non-photosensitive source of reducible silver ions, and

B) positioning one or more gold(III)-containing chemical sensitizers and one or more sulfur- or tellurium-containing chemical sensitizers on or around said photosensitive silver halide grains, said one or more gold(III)-containing chemical sensitizers being represented by the following Structure GOLD:



GOLD

50 wherein L' represents the same or different ligands, each ligand comprising at least one heteroatom that is capable of forming a bond with gold, Y is an anion, r is an integer of from 1 to 8, and q is an integer of from 0 to 3.

29. A method of preparing a photothermographic emulsion comprising:

A) providing photosensitive silver halide grains,

B) providing a photothermographic emulsion of said photosensitive silver halide grains and a non-photosensitive source of reducible silver ions, and

C) prior to, during, or immediately following either or both of steps A and B, chemically sensitizing said photosensitive silver halide grains with a combination of chemical sensitizers that consists essentially of a sulfur- or tellurium-containing compound, and a gold (III)-containing compound,

69

said gold(III)-containing compound being represented by the following Structure GOLD:

Au(III)L',Y<sub>q</sub>

GOLD

wherein L' represents the same or different ligands, each ligand comprising at least one heteroatom that is capable of forming a bond with gold, Y is an anion, r is an integer of from 1 to 8, and q is an integer of from 0 to 3.

30. The method of claim 29 wherein step C follows step B.

31. The method of claim 29 wherein step C is carried out between steps A and B.

32. The method of claim 29 wherein step C is carried out prior to step A.

33. The method of claim 29 wherein said combination of chemical sensitizers consists essentially of an organic sulfur-containing compound and said gold(III)-containing compound, and step C comprises decomposing said organic sulfur-containing compound on or around said photosensitive silver halide grains in an oxidizing environment.

34. The method of claim 33 wherein said organic sulfur-containing compound is a spectral sensitizing dye.

35. The method of claim 34 further comprising adding a second spectral sensitizing dye to said photothermographic emulsion to spectrally sensitize said photosensitive silver halide grains.

36. The method of claim 29 further comprising adding a reducing agent for said reducible silver ions to said photothermographic emulsion.

37. The method of claim 29 wherein the molar ratio of said sulfur- or tellurium-containing compound to said gold (III)-containing compound is from about 10,000:1 to about 1:10.

38. The method of claim 37 wherein the molar ratio of said sulfur- or tellurium-containing compound to said gold (III)-containing compound is from about 5,000:1 to about 1:1.

39. The method of claim 29 wherein said photosensitive silver halide grains are chemically sensitized with said sulfur- or tellurium-containing compound in an amount of from about 10<sup>-7</sup> to about 10<sup>-2</sup> mole per mole of total silver and with said gold(III)-containing compound in an amount of from about 10<sup>-8</sup> to about 10<sup>-2</sup> mole per mole of total silver.

40. A photothermographic material comprising a support having thereon one or more layers comprising a binder and in reactive association:

- photosensitive silver halide grains,
- a non-photosensitive source of reducible silver ions, and
- a reducing composition for said reducible silver ions, wherein said photosensitive silver halide grains have been chemically sensitized with a combination of chemical sensitizers that consists essentially of a combination of sulfur- and tellurium-containing compounds, and a gold(III)-containing compound that is represented by the following Structure GOLD:

Au(III)L',Y<sub>q</sub>

GOLD

wherein L' represents the same or different ligands, each ligand comprising at least one heteroatom that is capable of forming a bond with gold, Y is an anion, r is an integer of from 1 to 8, and q is an integer of from 0 to 3.

70

41. The photothermographic material of claim 40 wherein the tellurium-containing compound is represented by the following Structure I, II or III:



I

Te(L)<sub>m</sub>(X<sup>1</sup>)<sub>n</sub>

II

Pd(X<sup>2</sup>)<sub>2</sub>[Te(R)<sub>2</sub>]<sub>2</sub>

III

wherein X represents a COR, CSR, CN(R)<sub>2</sub>, CR, P(R)<sub>2</sub>, or P(OR)<sub>2</sub> group, R is an alkyl, alkenyl, or aryl group, L represents the same or different ligand derived from a neutral Lewis base, X<sup>1</sup> and X<sup>2</sup> represent a halo, OCN, SCN, S<sub>2</sub>CN(R)<sub>2</sub>, S<sub>2</sub>COR, S<sub>2</sub>CSR, S<sub>2</sub>P(OR)<sub>2</sub>, S<sub>2</sub>P(R)<sub>2</sub>, SeCN, TeCN, CN, SR, OR, N<sub>3</sub>, alkyl, aryl, or O<sub>2</sub>CR group, R' is an alkyl or aryl group, p is 2 or 4, m is 0, 1, 2, or 4, and n is 2 or 4, provided that when m is 0 or 2, n is 2 or 4, and when m is 1 or 4, n is 2.

42. The photothermographic material of claim 40 wherein said photosensitive silver halide is chemically sensitized with a sulfur-containing compound that is represented by the following Structure IV, V, or VI:



V



VI



wherein:

in Structure V, R<sub>1</sub>, R<sub>2</sub>, R<sub>3</sub> and R<sub>4</sub> are independently hydrogen, alkyl, cycloalkyl, allyl, alkenyl, alkynyl, aryl or heterocyclic groups, or R<sub>1</sub> and R<sub>2</sub> taken together, R<sub>3</sub> and R<sub>5</sub> taken together, R<sub>1</sub> and R<sub>3</sub> taken together or R<sub>2</sub> and R<sub>4</sub> taken together, can form a 5- to 7-membered heterocyclic ring,

in Structure V, R<sub>1</sub>, R<sub>2</sub>, R<sub>3</sub>, R<sub>4</sub> and R<sub>5</sub> are independently hydrogen, alkyl, cycloalkyl, allyl, alkenyl, alkynyl, aryl or heterocyclic groups, or R<sub>3</sub> and R<sub>5</sub> taken together, R<sub>4</sub> and R<sub>5</sub> taken together, R<sub>1</sub> and R<sub>3</sub> taken together or R<sub>2</sub> and R<sub>4</sub> taken together, can form a substituted or unsubstituted 5- to 7-membered heterocyclic ring, and

in Structure VI, R<sub>1</sub>, R<sub>2</sub>, R<sub>3</sub>, R<sub>4</sub>, R<sub>5</sub>, and R<sub>6</sub> are independently hydrogen, alkyl, cycloalkyl, allyl, alkenyl, alkynyl, aryl or heterocyclic groups, or R<sub>3</sub> and R<sub>6</sub> taken together, R<sub>4</sub> and R<sub>5</sub> taken together, R<sub>1</sub> and R<sub>3</sub> taken together, R<sub>2</sub> and R<sub>4</sub> taken together, or R<sub>5</sub> and R<sub>6</sub> taken together, can form a substituted or unsubstituted 5- to 7-membered heterocyclic ring, and R<sub>7</sub> is a divalent aliphatic or alicyclic linking group.

43. The photothermographic material of claim 40 wherein said photosensitive silver halide is chemically sensitized with a sulfur-containing compound containing a thiohydantoin, rhodanine, or the 2-thio-4-oxo-oxazolidine nucleus that is represented by the following Structure VII, VIII, or IX:



44. A photothermographic material comprising a support having thereon one or more layers comprising a binder and in reactive association:

- a. photosensitive silver halide grains,
- b. a non-photosensitive source of reducible silver ions, and
- c. a reducing composition for said reducible silver ions, wherein said photosensitive silver halide grains have been chemically sensitized with a combination of chemical sensitizers that consists essentially of a sulfur- or tellurium-containing compound, and a gold(III)-containing compound that is represented by the following Structure GOLD:

Au(III)L',Y<sub>q</sub>

GOLD

wherein L' represents the same or different bipyridine, terpyridine, P(phenyl)<sub>3</sub>, carboxylate, imine, phenol, mercaptophenol, imidazole, triazole, or dithioxamide

ligands, each ligand comprising at least one heteroatom that is capable of forming a bond with gold, Y is an anion, r is an integer of from 1 to 8, and q is an integer of from 0 to 3.

45. A photothermographic material comprising a support having thereon one or more layers that have been coated out of an organic solvent and comprises a binder, and in reactive association:

- a. photosensitive silver halide grains,
- b. a non-photosensitive source of reducible silver ions, and
- c. a reducing composition for said reducible silver ions, wherein said photosensitive silver halide grains have been chemically sensitized with a combination of chemical sensitizers that consists essentially of a sulfur- or tellurium-containing compound, and a gold(III)-containing compound that is represented by the following Structure GOLD:

Au(III)L',Y<sub>q</sub>

GOLD

wherein L' represents the same or different ligands, each ligand comprising at least one heteroatom that is capable of forming a bond with gold, Y is an anion, r is an integer of from 1 to 8, and q is an integer of from 0 to 3.

46. A photothermographic emulsion formulation comprising an organic solvent, a hydrophobic binder, photosensitive silver halide grains, a non-photosensitive source of reducible silver ions, and a reducing composition for said reducible silver ions,

wherein said photosensitive silver halide grains have been chemically sensitized with a combination of chemical sensitizers that consists essentially of a sulfur- or tellurium-containing compound, and a gold(III)-containing compound that is represented by the following Structure GOLD:

Au(III)L',Y<sub>q</sub>

GOLD

wherein L' represents the same or different ligands, each ligand comprising at least one heteroatom that is capable of forming a bond with gold, Y is an anion, r is an integer of from 1 to 8, and q is an integer of from 0 to 3.

\* \* \* \* \*